# EUROPEAN PATENT SPECIFICATION

(11) **EP 3 940 724 B1**
(45) Date of publication and mention of the grant of the patent: **11.12.2024**
(21) Application number: 20904841.2
(22) Date of filing: 07.07.2020
(51) Int. Cl.: H01F 1/057, H01F 41/02

(54) **PREPARATION METHOD FOR AN RTB-BASED PERMANENT MAGNET MATERIAL**
HERSTELLUNGSVERFAHREN FÜR EIN RTB-BASIERTES PERMANENTMAGNETMATERIAL
PROCÉDÉ DE PRÉPARATION POUR UN MATÉRIAU D'AIMANT PERMANENT À BASE DE RTB

(30) Priority: 24.12.2019 CN 201911348776
(43) Date of publication of application: 19.01.2022
(73) Proprietor: Fujian Golden Dragon Rare-Earth Co., Ltd., Longyan City, Fujian Province 366300 (CN)
(72) Inventor: HUANG, Qingfang, Longyan, Fujian 366300 (CN); FU, Gang, Longyan, Fujian 366300 (CN); CHEN, Dakun, Longyan, Fujian 366300 (CN); HUANG, Jiaying, Xiamen, Fujian 361000 (CN); XU, Deqin, Longyan, Fujian 366300 (CN); LIU, Shaowei, Longyan, Fujian 366300 (CN)
(74) Representative: karo IP
(86) International application number: PCT/CN2020/100580
(87) International publication number: WO 2021/128801

(56) References cited:
- EP-A2- 1 675 133
- EP-B1- 0 536 421
- CN-A- 1 723 511
- CN-A- 103 366 918
- CN-A- 103 745 823
- CN-A- 105 845 304
- CN-A- 105 845 304
- CN-A- 110 299 234
- CN-A- 110 428 947
- CN-A- 110 942 878
- CN-A- 110 993 232
- CN-C- 1 306 527
- JP-A- 2011 060 965
- JP-A- 2014 027 268
- JP-A- H02 285 604
- US-A1- 2017 323 722
- US-A1- 2018 277 288

## Description

### Technical Field

The present disclosure relates to an RTB-based permanent magnet material, a preparation method thereof, and an application thereof.

### Background

Since the Soviet scientists discovered Nd₂Fe₁₄B in 1979, the researchers in the United States and Japan took the lead in the study of the properties of the phase, the phase composed of PrNd (the mass ratio of Pr to Nd is 20 : 80 or 25 : 75) has been applied to the production of sintered permanent magnet in commercial at present, due to its advantages such as high magnetic energy product and high remanent magnetism, at present it has been widely used in motor, electroacoustic device, computer hard disk drive (HDD), military equipment, human nuclear magnetic resonance imaging (MRI), microwave communication technology, controller, instrument and so on.

With the progress of science and technology, higher requirements has been put forward for the performance of Nd-Fe-B, many researchers has improved the performance of neodymium-iron-boron magnet material by adding a large number of heavy rare earth Dy or Tb, however, excessive use of heavy rare earths will dramatically increase the cost of materials, and at the same time, the resources of heavy rare earths are relatively few.

Therefore, the technical problem to be solved urgently in this field is how to make use of the elements with abundant resources to obtain the neodymium-iron-boron material with high coercivity and high remanence.

In addition, how to achieve high uniformity and stability of magnetic properties of mass-produced magnets and control the production cost at the same time is also a problem that has been committed to solving in this field. However, carbon, sulfur, hydrogen, oxygen, nitrogen and other impurities will be inevitably introduced into the neodymium-iron-boron magnet material in the process, which poses a great challenge to the production of magnets with uniform and stable magnetic properties. In addition, it is generally believed in this field that the high content of carbon impurities will lead to the uneven grain size of the magnet's main phase and the uneven distribution of neodymium-rich phase, resulting in the decrease of various performance indexes of the magnet in different degrees. Therefore, in order to improve the uniformity stability of magnets, the production process need to be strictly controlled. CN 110 428 947 shows a similar production process to the present invention.

### Content of the present invention

The technical problem to be solved in the present invention is for overcoming the defects that the performance improvement of sintered neodymium-iron-boron magnet is excessively dependent on heavy rare earth elements in the prior art, while the high content of carbon element in sintered neodymium-iron-boron magnet will lead to the decrease of the performance of the magnet. Instead, the present invention provides an RTB-based permanent magnet material and a preparation method and an application thereof. The RTB-based permanent magnetic material provided by the invention can realize the improvement of the performance of permanent magnetic materials in the absence of heavy rare earth, and it is not necessary to control the content of carbon elements introduced in the process. Under the condition of high carbon content, the magnet still maintains excellent performance.

The present invention provides a method to produce an RTB-based permanent magnet material, which comprises the following components by mass percentage:
R': 29.5-33.5 wt.%, wherein: R' is a rare earth element and R' comprises Pr; the content of Pr is ≥ 8.85wt.%;
C: 0.106-0.26 wt.%;
O: ≤ 0.07 wt.%;
X: 0-5.0 wt.%, X is one or more of Cu, Al, Ga, Co, Zr, Ti, Nb and Mn;
B: 0.90-1.2 wt.%;
Fe: 61.4-69.5 wt.%.

In the present invention, the content of R' is 29.5-33.4 wt.%, such as, 29.5 wt.%, 30.5 wt.%, 30.8 wt.%, 31.0 wt.%, 31.013 wt.%, 31.075 wt.%, 31.115 wt.%, 31.5 wt.%, 32.0 wt.%, 32.3 wt.%, 32.8 wt.% or 33.3 wt.%, the percentage refers to the mass percentage in the RTB-based permanent magnet material.

In the present invention, the content of Pr is preferably 8.85-27.15 wt.%, more preferably ≥17.00 wt.%, such as, 8.846 wt.%, 8.848 wt.%, 8.849 wt.%, 8.851 wt.%, 9.852 wt.%, 10.148 wt.%, 10.151 wt.%, 10.848 wt.%, 10.849 wt.%, 11.848 wt.%, 12.148 wt.%, 12.15 wt.%, 12.151 wt.%, 13.149 wt.%, 14.147 wt.%, 14.148 wt.%, 14.149 wt.%, 14.151 wt.%, 14.152 wt.%, 16.148 wt.%, 16.151 wt.%, 16.152 wt.%, 17.148 wt.%, 17.149 wt.%, 17.15 wt.%, 17.151 wt.%, 17.152 wt.%, 18.148 wt.%, 18.149 wt.%, 18.151 wt.%, 18.152 wt.%, 19.148 wt.%, 19.149 wt.%, 19.15 wt.%, 19.151 wt.%, 19.152 wt.%, 20.148 wt.%, 20.149 wt.%, 20.15 wt.%, 20.152 wt.%, 21.148 wt.%, 22.149 wt.%, 22.151 wt.%, 23.149 wt.%, 23.15 wt.%, 24.148 wt.%, 24.151 wt.%, 24.152 wt.%, 25.152 wt.% or 27.148 wt.%, the percentage refers to the mass percentage in the RTB-based permanent magnet material.

In the present invention, R' can further comprise Nd and/or R, R is a rare earth element besides Pr and Nd.

Wherein, the content of Nd is preferably 3.3-23.0 wt.%, such as, 3.348 wt.%, 5.352 wt.%, 6.652 wt.%, 6.851 wt.%, 7.351 wt.%, 7.353 wt.%, 7.849 wt.%, 8.351 wt.%, 8.651 wt.%, 8.652 wt.%, 8.852 wt.%, 9.349 wt.%, 9.352 wt.%, 10.651 wt.%, 10.851 wt.%, 11.348 wt.%, 11.351 wt.%, 11.352 wt.%, 11.651 wt.%, 11.652 wt.%, 11.851 wt.%, 12.351 wt.%, 12.352 wt.%, 12.649 wt.%, 12.65 wt.%, 12.651 wt.%, 12.652 wt.%, 13.348 wt.%, 13.352 wt.%, 13.353 wt.%, 13.649 wt.%, 13.651 wt.%, 13.653 wt.%, 13.848 wt.%, 13.852 wt.%, 14.348 wt.%, 14.35 wt.%, 14.351 wt.%, 14.352 wt.%, 14.355 wt.%, 14.652 wt.%, 14.849 wt.%, 15.352 wt.%, 15.353 wt.%, 16.349 wt.%, 16.35 wt.%, 16.651 wt.%, 16.848 wt.%, 17.352 wt.%, 17.652 wt.%, 18.335 wt.%, 18.651 wt.%, 18.652 wt.%, 18.849 wt.%, 19.351 wt.%, 19.649 wt.%, 19.652 wt.%, 20.652 wt.%, 20.851 wt.%, 21.353 wt.%, 21.647 wt.%, 21.648 wt.%, 21.649 wt.%, 21.951 wt.%, 22.149 wt.% or 22.652 wt.%, the percentage refers to the mass percentage in the RTB-based permanent magnet material.

Wherein, the mass ratio of Nd to R' is preferably ≤0.72, more preferably <0.5; such as, 0.110, 0.175, 0.216, 0.221, 0.233, 0.241, 0.253, 0.281, 0.283, 0.286, 0.297, 0.307, 0.317, 0.346, 0.350, 0.360, 0.366, 0.372, 0.378, 0.382, 0.385, 0.392, 0.395, 0.411, 0.416, 0.422, 0.424, 0.438, 0.443, 0.447, 0.456, 0.470, 0.476, 0.479, 0.487, 0.520, 0.536, 0.541, 0.544, 0.551, 0.554, 0.588, 0.598, 0.601, 0.606, 0.608, 0.614, 0.632, 0.644, 0.666, 0.671, 0.673, 0.678, 0.696, 0.697, 0.700, 0.710, 0.713, 0.714, 0.715 or 0.719.

Wherein, the kind of R is preferably Y and/or Ce.

Wherein, the content of R is preferably 0-1 wt.%, such as, 0.29 wt.%, the percentage refers to the mass percentage in the RTB-based permanent magnet material.

In the present invention, R' comprises a heavy rare earth element RH.

Wherein, the kind of RH can be Dy and/or Tb.

Wherein, the content of RH can be the conventional content in this field, the content of RH is preferably 0.5-2.6 wt.%, such as 0.58 wt.% , 0.62 wt.%, 1.212 wt.%, 1.219 wt.%, 1.51 wt.%, 1.991 wt.%, 2.011 wt.%, 2.511 wt.% or 2.512 wt.%, the percentage refers to the mass percentage of the RTB-based permanent magnet material.

Wherein, the mass ratio of RH to R is preferably <0.253, for example 0.019-0.075, such as 0.019, 0.020, 0.038, 0.039, 0.047, 0.061 or 0.075.

When the RH comprises Tb, the content of Tb is preferably 0.5-2.0 wt.%, such as 1.991 wt.%, 1.212 wt.%, 1.219 wt.% or 0.58 wt.%, the percentage refers to the mass percentage in the RTB-based permanent magnet material.

When the RH comprises Dy, the content of Dy is preferably 0.6-2.52 wt.%, such as 0.62 wt.%, 1.51 wt.%, 2.011 wt.%, 2.511 wt.%, or 2.512 wt.%, and the percentage refers to the mass percentage in the RTB-based permanent magnet material.

In the present invention, the content of C is 0.106-0.25 wt.%, such as, 0.1062 wt.%, 0.1069 wt.%, 0.1072 wt.%, 0.1075 wt.%, 0.1251 wt.%, 0.1253 wt.%, 0.1256 wt.%, 0.1532 wt.%, 0.1534 wt.%, 0.1537 wt.%, 0.1759 wt.%, 0.1761 wt.%, 0.1764 wt.%, 0.1835 wt.%, 0.184 wt.%, 0.1843 wt.%, 0.1846 wt.%, 0.1965 wt.%, 0.197 wt.%, 0.1973 wt.%, 0.2139 wt.%, 0.2144 wt.%, 0.2147 wt.%, 0.2243 wt.%, 0.2245 wt.%, 0.2248 wt.%, 0.2251 wt.%, 0.2379 wt.% or 0.2456 wt.%, the percentage refers to the mass percentage in the RTB-based permanent magnet material.

In the present invention, the content of O is ≤0.0691 wt.%, such as 0.0382 wt.%, 0.0384 wt.%, 0.039 wt.%, 0.0391 wt.%, 0.041 wt.%, 0.0412 wt.%, 0.0432 wt.%, 0.0442 wt.%, 0.0444 wt.%, 0.0456 wt.%, 0.0458 wt.%, 0.0468 wt.%, 0.0492 wt.%, 0.0493 wt.%, 0.0494 wt.%, 0.05 wt.%, 0.0501 wt.%, 0.0503 wt.%, 0.0523 wt.%, 0.0529 wt.%, 0.0531 wt.%, 0.0558 wt.%, 0.0564 wt.%, 0.0566 wt.%, 0.0582 wt.%, 0.0588 wt.%, 0.059 wt.%, 0.0635 wt.%, 0.0641 wt.%, 0.0643 wt.%, 0.0669 wt.%, 0.0675 wt.%, 0.0685 wt.% or 0.0691 wt.%, the percentage refers to the mass percentage in the RTB-based permanent magnet material.

In the present invention, the content of B is 0.94-1.1 wt.%, such as, 0.946 wt.%, 0.947 wt.%, 0.948 wt.%, 0.949 wt.%, 0.951 wt.%, 0.952 wt.%, 0.958 wt.%, 0.961 wt.%, 0.962 wt.%, 0.981 wt.%, 0.982 wt.%, 0.985 wt.%, 0.998 wt.%, 1.008 wt.%, 1.009 wt.%, 1.01 wt.%, 1.011 wt.% or 1.012 wt.%, the percentage refers to the mass percentage in the RTB-based permanent magnet material.

In the present invention, the content of Fe is 61.4-69.3 wt.%, such as, 61.49 wt.%, 61.60 wt.%, 62.15 wt.%, 62.19 wt.%, 62.66 wt.%, 62.91 wt.%, 63.52 wt.%, 63.62 wt.%, 63.66 wt.%, 64.71 wt.%, 65.85 wt.%, 66.02 wt.%, 66.15 wt.%, 66.19 wt.%, 66.22 wt.%, 66.23 wt.%, 66.30 wt.%, 66.37 wt.%, 66.40 wt.%, 66.44 wt.%, 66.57 wt.%, 66.66 wt.%, 66.70 wt.%, 66.72 wt.%, 66.75 wt.%, 66.82 wt.%, 66.85 wt.%, 66.88 wt.%, 66.91 wt.%, 66.94 wt.%, 66.95 wt.%, 66.98 wt.%, 67.08 wt.%, 67.15 wt.%, 67.17 wt.%, 67.23 wt.%, 67.27 wt.%, 67.29 wt.%, 67.30 wt.%, 67.31 wt.%, 67.32 wt.%, 67.34 wt.%, 67.40 wt.%, 67.42 wt.%, 67.47 wt.%, 67.48 wt.%, 67.54 wt.%, 67.64 wt.%, 67.65 wt.%, 67.69 wt.%, 67.71 wt.%, 67.74 wt.%, 67.78 wt.%, 67.80 wt.%, 68.22 wt.%, 68.24 wt.%, 68.25 wt.%, 68.27 wt.%, 68.28 wt.%, 68.31 wt.%, 68.32 wt.%, 68.34 wt.%, 68.36 wt.%, 68.73 wt.%, 68.83 wt.%, 68.95 wt.%, 69.03 wt.%, 69.10 wt.% or 69.25 wt.%, the percentage refers to the mass percentage in the RTB-based permanent magnet material.

In the present invention, X can be Cu, Al, Ga, Co, Zr, Ti or Nb, can also be "Cu and Al", "Ga and Mn", " Cu, Al and Ga", "Cu, Al, Ga and Zr", "Cu, Al, Ga and Co" or "Cu, Al, Ga, Zr and Co".

In the present invention, the content of X is preferably 0-4.5 wt.%, such as, 0.021 wt.%, 0.041 wt.%, 0.101 wt.%, 0.102 wt.%, 0.201 wt.%, 0.202 wt.%, 0.251 wt.%, 0.301 wt.%, 0.302 wt.%, 0.351 wt.%, 0.352 wt.%, 0.362 wt.%, 0.401 wt.%, 0.421 wt.%, 0.423 wt.%, 0.451 wt.%, 0.497 wt.%, 0.5 wt.%, 0.501 wt.%, 0.523 wt.%, 0.526 wt.%, 0.601 wt.%, 0.602 wt.%, 0.643 wt.%, 0.673 wt.%, 0.702 wt.%, 0.704 wt.%, 0.743 wt.%, 0.801 wt.%, 0.803 wt.%, 0.871 wt.%, 0.882 wt.%, 0.894 wt.%, 0.901 wt.%, 0.945 wt.%, 1.021 wt.%, 1.022 wt.%, 1.105 wt.%, 1.194 wt.%, 1.274 wt.%, 1.305 wt.%, 1.402 wt.%, 1.506 wt.%, 1.562 wt.%, 1.732 wt.%, 1.905 wt.%, 2.501 wt.%, 3.803 wt.%, 3.809 wt.%, 3.813 wt.%, 3.814 wt.%, 3.865 wt.%, 3.959 wt.%, 4.199 wt.%, 4.207 wt.% or 4.208 wt.%, the percentage refers to the mass percentage in the RTB-based permanent magnet material.

When X comprises Cu, the content of Cu is preferably 0.2-0.51 wt.%, such as, 0.201 wt.%, 0.302 wt.%, 0.34 wt.%, 0.341 wt.%, 0.351 wt.%, 0.381 wt.%, 0.382 wt.%, 0.4 wt.%, 0.401 wt.%, 0.402 wt.%, 0.403 wt.%, 0.41 wt.%, 0.42 wt.%, 0.421 wt.%, 0.441 wt.%, 0.451 wt.%, 0.5 wt.%, 0.501 wt.% or 0.502 wt.%, the percentage refers to the mass percentage in the RTB-based permanent magnet material.

When X comprises Al, the content of Al is preferably 0-0.81 wt.%, but not 0, for example, 0.01-0.03 wt.% or 0.5-0.8 wt.%, such as 0.01 wt.%, 0.021 wt.%, 0.03 wt.%, 0.041 wt.%, 0.042 wt.%, 0.101 wt.%, 0.102 wt.%, 0.103 wt.%, 0.202 wt.%, 0.298 wt.%, 0.301 wt.%, 0.302 wt.%, 0.351 wt.%, 0.401 wt.%, 0.402 wt.%, 0.403 wt.%, 0.451 wt.%, 0.497 wt.%, 0.501 wt.%, 0.502 wt.%, 0.601 wt.%, 0.602 wt.%, 0.70 wt.2%, 0.801 wt.%, 0.802 wt.% or 0.81 wt.%, the percentage refers to the mass percentage in the RTB-based permanent magnet material.

When X comprises Ga, the content of Ga is preferably 0.0-1.85 wt.%, but not 0, more preferably 0.1-1.552 wt.%, such as 0.102 wt.%, 0.151 wt.%, 0.202 wt.%, 0.251 wt.%, 0.3 wt.%, 0.301 wt.%, 0.302 wt.%, 0.399 wt.%, 0.401 wt.%, 0.42 wt.%, 0.421 wt.%, 0.501 wt.%, 0.502 wt.%, 0.901 wt.%, 1.402 wt.% or 1.552 wt.%, the percentage refers to the mass percentage in the RTB-based permanent magnet material.

When X comprises Co, the content of Co is preferably 0.0-3.0 wt.%, but not 0, more preferably 0.5-2.5 wt.%, such as 0.5 wt.%, 1.0 wt.%, or 2.5 wt.%, the percentage refers to the mass percentage in the RTB-based permanent magnet material.

When X comprises Zr, the content of Zr is preferably 0.25-0.35 wt.%, such as 0.25 wt.%, 0.30 wt.% or 0.35 wt.%, the percentage refers to the mass percentage in the RTB-based permanent magnet material.

When X comprises Nb, the content of Nb is preferably 0.25-0.35 wt.%, such as 0.25 wt.%, 0.30 wt.% or 0.35 wt.%, the percentage refers to the mass percentage in the RTB-based permanent magnet material.

When X comprises Mn, the content of Mn is preferably 0.0-0.03 wt.%, but not 0, such as 0.01 wt.%, the percentage refers to the mass percentage in the RTB-based permanent magnet material.

In the present invention, the RTB-based permanent magnet material can further comprise conventional added element M, and for example, M is one or more selected from the group consisting of of Ni, Zn, Ag, In, Sn, Bi, V, Cr, Hf, Ta, and W.

Wherein, the kind of M is preferably Cr.

Wherein, the content of M is preferably 0-0.15 wt.%, but not 0, such as 0.05 wt.% or 0.12 wt.%, the percentage refers to the mass percentage in the RTB-based permanent magnet material.

In the present invention, the RTB-based permanent magnet material can further comprise nitrogen element N, preferably, the content of N is ≤0.05 wt.%, such as 0.0182 wt.%, 0.0187 wt.%, 0.0223 wt.%, 0.0228 wt.%, 0.025 wt.%, 0.0251 wt.%, 0.0256 wt.%, 0.0284 wt.%, 0.0285 wt.%, 0.029 wt.%, 0.0301 wt.%, 0.0302 wt.%, 0.0307 wt.%, 0.0341 wt.%, 0.0342 wt.%, 0.0347 wt.%, 0.0366 wt.%, 0.0371 wt.%, 0.0372 wt.%, 0.0375 wt.%, 0.0378 wt.%, 0.0397 wt.%, 0.0398 wt.%, 0.0401 wt.%, 0.0404 wt.%, 0.0436 wt.%, 0.0439 wt.%, 0.0442 wt.%, 0.0455 wt.%, 0.0458 wt.%, 0.0461 wt.%, 0.0476 wt.%, 0.0482 wt.%, 0.0485 wt.% or 0.0486 wt.%, the percentage refers to the mass percentage in the RTB-based permanent magnet material.

In a preferred embodiment of the present invention, the RTB-based permanent magnet material comprises the following components: R': 29.5-33.5 wt.%, Pr ≥ 8.85 wt.%, C: 0.106-0.25 wt.%, O: ≤0.07 wt.%, B: 0.94-1.1 wt.%, Fe: 61.4-69.3 wt.%, the percentage refers to the mass percentage in the RTB-based permanent magnet material.

In a preferred embodiment of the present invention, the RTB-based permanent magnet material comprises the following components: R': 29.5-33.5 wt.%, Pr ≥ 8.85 wt.%, C: 0.106-0.25 wt.%, O: ≤0.07 wt.%, Cu: 0.2-0.51 wt.%, B: 0.94-1.1 wt.%, Fe: 61.4-69.3 wt.%, the percentage refers to the mass percentage in the RTB-based permanent magnet material.

In a preferred embodiment of the present invention, the RTB-based permanent magnet material comprises the following components: R': 29.5-33.5 wt.%, Pr ≥ 8.85 wt.%, C: 0.106-0.25 wt.%, O: ≤0.07 wt.%, Al: 0-0.81 wt.%, but not 0, B: 0.94-1.1 wt.%, Fe: 61.4-69.3 wt.%, the percentage refers to the mass percentage in the RTB-based permanent magnet material.

In a preferred embodiment of the present invention, the RTB-based permanent magnet material comprises the following components: R': 29.5-33.5 wt.%, Pr > 8.85 wt.%, C:0.106-0.25 wt.%, O: ≤0.07 wt.%, Ga: 0.1-1.85 wt.%, B: 0.94-1.1 wt.%, Fe: 61.4-69.3 wt.%, the percentage refers to the mass percentage in the RTB-based permanent magnet material.

In a preferred embodiment of the present invention, the RTB-based permanent magnet material comprises the following components: R': 29.5-33.5 wt.%, Pr ≥ 8.85 wt.%, C: 0.106-0.25 wt.%, O: ≤ 0.07 wt.%, Co: 0.0-3.0 wt.%, but not 0, B: 0.94-1.1 wt.%, Fe: 61.4-69.3 wt.%, the percentage refers to the mass percentage in the RTB-based permanent magnet material.

In a preferred embodiment of the present invention, the RTB-based permanent magnet material comprises the following components: R': 29.5-33.5 wt.%, Pr ≥ 8.85 wt.%, C:0.106-0.25 wt.%, O: ≤ 0.07 wt.%, Zr: 0.25-0.35 wt.%, B: 0.94-1.1 wt.%, Fe: 61.4-69.3 wt.%, the percentage refers to the mass percentage in the RTB-based permanent magnet material.

In a preferred embodiment of the present invention, the RTB-based permanent magnet material comprises the following components: R': 29.5-33.5 wt.%, Pr ≥ 8.85 wt.%, C: 0.106-0.25 wt.%, O: ≤ 0.07 wt.%, Nb: 0.25-0.35 wt.%, B: 0.94-1.1 wt.%, Fe: 61.4-69.3 wt.%, the percentage refers to the mass percentage in the RTB-based permanent magnet material.

In a preferred embodiment of the present invention, the RTB-based permanent magnet material comprises the following components: R': 29.5-33.5 wt.%, Pr ≥ 8.85 wt.%, C: 0.106-0.25 wt.%, O: ≤ 0.07 wt.%, Cu: 0.34-0.51 wt.%, Al: 0-0.81 wt.%, but not 0, B: 0.94-1.1 wt.%, Fe: 61.4-69.3 wt.%, the percentage refers to the mass percentage in the RTB-based permanent magnet material.

In a preferred embodiment of the present invention, the RTB-based permanent magnet material comprises the following components: R': 29.5-33.5 wt.%, Pr ≥ 8.85 wt.%, C: 0.106-0.25 wt.%, O: ≤ 0.07 wt.%, Cu: 0.34-0.51 wt.%, Al: 0-0.81 wt.%, but not 0, Ga: 0.1-0.5 wt.%, B: 0.94-1.1 wt.%, Fe: 61.4-69.3 wt.%, the percentage refers to the mass percentage in the RTB-based permanent magnet material.

In a preferred embodiment of the present invention, the RTB-based permanent magnet material comprises the following components: R': 29.5-33.5 wt.%, Pr ≥ 8.85 wt.%, C: 0.106-0.25 wt.%, O: ≤ 0.07 wt.%, Cu: 0.34-0.51 wt.%, Al: 0.25-0.81 wt.%, Ga: 0.1-0.42 wt.%, Zr: 0.25-0.30 wt.%, B: 0.94-1.1 wt.%, Fe: 61.4-69.3 wt.%, the percentage refers to the mass percentage in the RTB-based permanent magnet material.

In a preferred embodiment of the present invention, the RTB-based permanent magnet material comprises the folloing components: R': 29.5-33.5 wt.%, Pr ≥ 8.85 wt.%, C:0.106-0.25 wt.%, O: ≤ 0.07 wt.%, Cu: 0.34-0.51 wt.%, Al: 0.25-0.81 wt.%, Ga: 0.1-0.41 wt.%, Co: 0.0-3.0 wt.%, Zr: 0.25-0.30 wt.%, Cr: 0.05-0.12 wt.%, B: 0.94-1.1 wt.%, Fe: 61.4-69.3 wt.%, the percentage refers to the mass percentage in the RTB-based permanent magnet material.

In a preferred embodiment of the present invention, the RTB-based permanent magnet material comprises the following components: R': 29.5-33.5 wt.%, Pr ≥ 8.85 wt.%, RH: 0.5-2.6 wt.%, C: 0.106-0.25 wt.%, O: ≤ 0.07 wt.%, Cu: 0.34-0.51 wt.%, Al: 0.25-0.81 wt.%, Ga: 0.1-0.41 wt.%, Co: 0.0-3.0 wt.%, Zr: 0.25-0.30 wt.%, B: 0.94-1.1 wt.%, Fe: 61.4-69.3 wt.%, the percentage refers to the mass percentage in the RTB-based permanent magnet material.

In a preferred embodiment of the present invention, the RTB-based permanent magnet material comprises the following components: R': 29.5-33.5 wt.%, Pr ≥ 8.85 wt.%, Ce: 0-1 wt.%, RH: 0.5-2.6 wt.%, C: 0.106-0.25 wt.%, O: ≤ 0.07 wt.%, Cu: 0.34-0.51 wt.%, Al: 0.25-0.81 wt.%, Ga: 0.1-0.41 wt.%, Co: 0.0-3.0 wt.%, Zr: 0.25-0.30 wt.%, B: 0.94-1.1 wt.%, Fe: 61.4-69.3 wt.%, the percentage refers to the mass percentage in the RTB-based permanent magnet material.

In the present invention, the RTB-based permanent magnet material generally includes a main phase, a grain boundary phase, and an intergranular triangle region, wherein, the intergranular triangle region is also called rare earth-rich phase.

Wherein, preferably, the percentage of the volume of the intergranular triangle region with respect to the sum of the volume of the "main phase, the grain boundary phase and the intergranular triangle region" is ≤9.0%, such as 3.2%, 3.3%, 3.7%, 4.6%, 4.8% or 5.3%.

Wherein, preferably, the content of rare earth elements in the intergranular triangle region is 84.35-85.85%, such as 84.35%, 84.8%, 84.9 %, 85%, 85.2%, 85.3%, 85.4% or 85.85%, and the percentage refers to the mass percentage in the total mass of elements in the intergranular triangle region.

Wherein, preferably, the content of O element in the intergranular triangle region is 13.25-14.8%, such as 13.25%, 13.7%, 14.2%, 14.3%, 14.4%, 14.5%, 14.6%, 14.7%, 14.75% or 14.8%, the percentage refers to the mass percentage in the total mass of the elements in the intergranular triangle region.

When the RTB-based permanent magnet material includes Cu, preferably, in the intergranular triangle region, the content of Cu element is 0.6-0.9%, such as 0.6, 0.8 or 0.9%, and the percentage refers to the mass percentage in the total mass of the elements in the intergranular triangle region.

When the RTB-based permanent magnet material includes Ga, preferably, in the intergranular triangle region, the content of Ga elements is 0.4-0.6%, such as 0.4% or 0.6%, and the percentage refers to the mass percentage in the total mass of the elements in the intergranular trigonal region.

When the RTB-based permanent magnet material includes Cu and Ga, preferably, in the intergranular triangle region, the content of Cu element is 0.3-0.4% and the content of Ga element is 0.5-0.6% such as 0.3% Cu, 0.6% Ga, 0.4% Cu, 0.4% Ga, 0.4% Cu, 0.5% Ga, or, 0.4% Cu, 0.6% Ga, the percentage refers to the mass percentage in the total mass of the elements in the intergranular triangle region.

The present invention as specified in claim provides a preparation method for RTB-based permanent magnet material, which comprises the following steps: the molten liquid of the raw material composition of the RTB-based permanent magnet material is subjected to casting, hydrogen decrepitation and pulverization to obtain a powder, and the powder is mixed with dispersant, and then pressed, formed, sintered and aged; wherein:
(1) the raw material composition of RTB-based permanent magnet material comprises the following components by mass percentage:
   R': 29.5-33.5 wt.%, R' is a rare earth element, R' comprises Pr, the content of Pr is ≥8.85 wt.%;
   X: 0-5.0 wt.%, X is one or more selected from the group consisting of Cu, Al, Ga, Co, Zr, Ti, Nb and Mn;
   B: 0.90-1.2 wt.%;
   Fe: 61.4-69.5 wt.%;
(2) in the process of pulverization, O ≤ 60 ppm in the pulverization atmosphere;
(3) in the pressing process, O ≤ 40 ppm in the pressing atmosphere;
(4) the dispersant comprises element C, and the mass percentage of the dispersant in the mixed powder is 0.04-0.2%.

In the present invention, the content of R' is preferably 29.5-33.3 wt.%, more preferably 9.5 wt.%, 30.5 wt.%, 30.8 wt.%, 31 wt.%, 31.5 wt.%, 32 wt.%, 32.3 wt.%, 32.8 wt.% or 33.3 wt.%, the percentage refers to the mass percentage in the raw material composition of the RTB-based permanent magnet material.

In the present invention, the content of Pr is preferably 8.85-27.15 wt.%, such as 8.85 wt.%, 9.85 wt.%, 10.15 wt.%, 10.85 wt.%, 11.85 wt.%, 12.15 wt.%, 13.15 wt.%, 14.15 wt.%, 16.15 wt.%, 17.15 wt.%, 18.15 wt.%, 19.15 wt.%, 20.15 wt.%, 21.15 wt.%, 22.15 wt.%, 23.15 wt.%, 24.15 wt.%, 25.15 wt.% or 27.15 wt.%, the percentage refers to the mass percentage in the raw material composition of the RTB-based permanent magnet material.

In the present invention, R' can further comprise Nd and/or R, R is a rare earth element besides Pr and Nd.

Wherein, the content of Nd is preferably 3.35-22.65 wt.%, more preferably 3.35 wt.%, 5.35 wt.%, 6.65 wt.%, 6.85 wt.%, 7.35 wt.%, 7.85 wt.%, 8.35 wt.%, 8.65 wt.%, 8.85 wt.%, 9.35 wt.%, 10.65 wt.%, 10.85 wt.%, 11.35 wt.%, 11.65 wt.%, 11.85 wt.%, 12.35 wt.%, 12.65 wt.%, 13.35 wt.%, 13.65 wt.%, 13.85 wt.%, 14.35 wt.%, 14.65 wt.%, 14.8 wt.5%, 15.35 wt.%, 16.35 wt.%, 16.65 wt.%, 16.85 wt.%, 17.35 wt.%, 17.65 wt.%, 18.35 wt.%, 18.65 wt.%, 18.85 wt.%, 19.35 wt.%, 19.65 wt.%, 20.65 wt.%, 20.85 wt.%, 21.35 wt.%, 21.65 wt.%, 21.95 wt.%, 22.15 wt.% or 22.65 wt.%, the percentage refers to the mass percentage in the raw material composition of the RTB-based permanent magnet material.

Wherein, the mass ratio of Nd to R' is preferably ≤0.72; such as, 0.11, 0.18, 0.22, 0.23, 0.24, 0.25, 0.28, 0.29, 0.30, 0.31, 0.32, 0.35, 0.36, 0.37, 0.38, 0.39, 0.40, 0.41, 0.42, 0.44, 0.45, 0.46, 0.47, 0.48, 0.49, 0.52, 0.54, 0.55, 0.59, 0.60, 0.61, 0.63, 0.64, 0.67, 0.68, 0.70 or 0.72.

Wherein, the kind of R is preferably Y and/or Ce.

Wherein, the content of R is preferably 0-1 wt.%, for example 0.3 wt.%, the percentage refers to the mass percentage in the raw material composition of the RTB-based permanent magnet material.

In the present invention, R' comprises a heavy rare earth element RH.

Wherein, the kind of RH can be Dy and/or Tb.

Wherein, the content of RH can be the conventional content in this field, preferably 1.2-2.5 wt.%, such as 1.2 wt.%, 1.5 wt.%, 2 wt.% or 2.5 wt.%, and the percentage refers to the mass percentage in the raw material composition of the RTB-based permanent magnet material.

Wherein, the mass ratio of RH to R' is preferably < 0.253, for example 0.038-0.075, such as 0.038, 0.039, 0.046, 0.061 or 0.075.

When the RH comprises Tb, the content of Tb is preferably 1.2-2.0 wt.%, for example 1.2 wt.% or 2.0 wt.%, the percentage refers to the mass percentage in the raw material composition of the RTB-based permanent magnet material.

When the RH comprises Dy, the content of Dy is preferably 1.5-2.5 wt.%, such as 1.5 wt.%, 2.0 wt.% or 2.5 wt.%, the percentage refers to the mass percentage in the raw material composition of the RTB-based permanent magnet material.

In the present invention, the content of B is preferably 0.95-1.1 wt.%, such as 0.95 wt.%, 0.96 wt.%, 0.98 wt.% or 1.01 wt.%, the percentage refers to the mass percentage in the raw material composition of the RTB-based permanent magnet material.

In the present invention, the content of Fe is preferably 61.5-69.5 wt.%, such as 61.79 wt.%, 61.89 wt.%, 62.44 wt.%, 62.89 wt.%, 63.24 wt.%, 63.84 wt.%, 63.87 wt.%, 63.94 wt.%, 64.99 wt.%, 66.19 wt.%, 66.29 wt.%, 66.47 wt.%, 66.52 wt.%, 66.55 wt.%, 66.61 wt.%, 66.69 wt.%, 66.75 wt.%, 66.85 wt.%, 66.97 wt.%, 67.00 wt.%, 67.02 wt.%, 67.068 wt.%, 67.13 wt.%, 67.14 wt.%, 67.19 wt.%, 67.24 wt.%, 67.25 wt.%, 67.35 wt.%, 67.37 wt.%, 67.45 wt.%, 67.49 wt.%, 67.54 wt.%, 67.55 wt.%, 67.57 wt.%, 67.59 wt.%, 67.64 wt.%, 67.65 wt.%, 67.69 wt.%, 67.718 wt.%, 67.75 wt.%, 67.85 wt.%, 67.95 wt.%, 67.96 wt.%, 67.97 wt.%, 68.008 wt.%, 68.12 wt.%, 68.55 wt.%, 68.62 wt.%, 69.02 wt.%, 69.1 wt.%, 69.22 wt.%, 69.27 wt.%, 69.32 wt.% or 69.45 wt.%, the percentage refers to the mass percentage in the raw material composition of the RTB-based permanent magnet material.

In the present invention, X can be Cu, Al, Ga, Co, Zr, Ti or Nb, can also be "Cu and Al", "Ga and Mn", "Cu, Al and Ga", "Cu, Al, Ga and Zr", "Cu, Al, Ga and Co" or "Cu, Al, Ga, Zr and Co".

In the present invention, the content of the X is preferably 0-4.5 wt.%, such as, 0.02 wt.%, 0.042 wt.%, 0.1 wt.%, 0.2 wt.%, 0.25 wt.%, 0.3 wt.%, 0.35 wt.%, 0.36 wt.%, 0.4 wt.%, 0.42 wt.%, 0.422 wt.%, 0.45 wt.%, 0.5 wt.%, 0.52 wt.%, 0.522 wt.%, 0.6 wt.%, 0.64 wt.%, 0.67 wt.%, 0.7 wt.%, 0.74 wt.%, 0.8 wt.%, 0.87 wt.%, 0.88 wt.%, 0.89 wt.%, 0.9 wt.%, 0.94 wt.%, 1.00 wt.%, 1.02 wt.%, 1.1 wt.%, 1.19 wt.%, 1.27 wt.%, 1.3 wt.%, 1.4 wt.%, 1.5 wt.%, 1.56 wt.%, 1.72 wt.%, 1.9 wt.%, 2.5 wt.%, 3.8 wt.%, 3.85 wt.%, 3.95 wt.% or 4.2 wt.%, the percentage refers to the mass percentage in the raw material composition of the RTB-based permanent magnet material.

When X comprises Cu, the content of the Cu is preferably 0.2-0.5 wt.%, such as, 0.2 wt.%, 0.3 wt.%, 0.34 wt.%, 0.35 wt.%, 0.38 wt.%, 0.4 wt.%, 0.42 wt.%, 0.44 wt.%, 0.45 wt.% or 0.5 wt.%, the percentage refers to the mass percentage in the raw material composition of the RTB-based permanent magnet material.

When the X comprises Al, the content of Al is preferably 0-0.8 wt.%, but not 0, such as 0.01-0.03 wt.% or 0.5-0.8 wt.%, and then 0.01 wt.%, 0.02 wt.%, 0.03 wt.%, 0.042 wt.%, 0.1 wt.%, 0.2 wt.%, 0.3 wt.%, 0.35 wt.%, 0.4 wt.%, 0.45 wt.%, 0.5 wt.%, 0.6 wt.%, 0.7 wt.% or 0.8 wt.%, the percentage refers to the mass percentage in the raw material composition of the RTB-based permanent magnet material.

When the X comprises Ga, the content of Ga is preferably 0.0-1.85 wt.%, but not 0, and more preferably 0.1-1.55 wt.%, such as, 0.1 wt.%, 0.15 wt.%, 0.2 wt.%, 0.25 wt.%, 0.3 wt.%, 0.4 wt.%, 0.42 wt.%, 0.5 wt.%, 0.9 wt.%, 1.4 wt.% or 1.55 wt.%, the percentage refers to the mass percentage in the raw material composition of the RTB-based permanent magnet material.

When the X comprises Co, the content of Co is preferably 0.0-3.0 wt.%, but not 0, and more preferably 0.5-2.5 wt.%, such as 0.5 wt.%, 1.0 wt.% or 2.5 wt.%, the percentage refers to the mass percentage in the raw material composition of the RTB-based permanent magnet material.

When the X comprises Zr, the content of Zr is preferably 0.25-0.35 wt.%, such as 0.25 wt.%, 0.30 wt.% or 0.35 wt.%, the percentage refers to the mass percentage in the raw material composition of the RTB-based permanent magnet material.

When the X comprises Nb, the content of Nb is preferably 0.25-0.35 wt.%, such as 0.25 wt.%, 0.30 wt.% or 0.35 wt.%, the percentage refers to the mass percentage in the raw material composition of the RTB-based permanent magnet material.

When the X comprises Mn, the content of Mn is preferably 0.0-0.03 wt.%, but not 0, such as 0.01 wt.%, the percentage refers to the mass percentage in the raw material composition of the RTB-based permanent magnet material.

In the present invention, the RTB-based permanent magnet material can further comprise conventional added element M, for example, M is one or more selected from the group of Ni, Zn, Ag, In, Sn, Bi, V, Cr, Hf, Ta and W.

Wherein, the kind of M is preferably Cr.

Wherein, the content of M is preferably 0-0.15 wt.%, but not 0, such as 0.05 wt.% or 0.12 wt.%, and the percentage refers to the mass percentage in the raw material composition of the RTB-based permanent magnet material.

In a preferred embodiment of the present invention, the raw material composition of the RTB-based permanent magnet material comprises the following components: R': 29.5-33.5 wt.%, Pr ≥ 8.85 wt.%, Cu: 0.2-0.5 wt.%, B: 0.95-1.1 wt.%, Fe: 61.5-69.5 wt.%, the percentage refers to the mass percentage in the raw material composition of the RTB-based permanent magnet material.

In a preferred embodiment of the present invention, the raw material composition of the RTB-based permanent magnet material comprises the following components: R': 29.5-33.5 wt.%, Pr ≥ 8.85 wt.%, Al: 0-0.8 wt.%, but not 0, B: 0.95-1.1 wt.%, Fe: 61.5-69.5 wt.%, the percentage refers to the mass percentage in the raw material composition of the RTB-based permanent magnet material.

In a preferred embodiment of the present invention, the raw material composition of the RTB-based permanent magnet material comprises the following components: R': 29.5-33.5 wt.%, Pr ≥ 8.85 wt.%, Ga: 0.1-1.85 wt.%, B: 0.95-1.1 wt.%, Fe: 61.5-69.5 wt.%, the percentage refers to the mass percentage in the raw material composition of the RTB-based permanent magnet material.

In a preferred embodiment of the present invention, the raw material composition of the RTB-based permanent magnet material comprises the following components: R': 29.5-33.5 wt.%, Pr ≥ 8.85 wt.%, Co: 0.0-3.0 wt.%, but not 0, B: 0.95-1.1 wt.%, Fe: 61.5-69.5 wt.%, the percentage refers to the mass percentage in the raw material composition of the RTB-based permanent magnet material.

In a preferred embodiment of the present invention, the raw material composition of the RTB-based permanent magnet material comprises the following components: R': 29.5-33.5 wt.%, Pr ≥ 8.85 wt.%, Zr: 0.25-0.35 wt.%, B: 0.95-1.1 wt.%, Fe: 61.5-69.5 wt.%, the percentage refers to the mass percentage in the raw material composition of the RTB-based permanent magnet material.

In a preferred embodiment of the present invention, the raw material composition of the RTB-based permanent magnet material comprises the following components: R': 29.5-33.5 wt.%, Pr ≥ 8.85 wt.%, Nb: 0.25-0.35 wt.%, B: 0.95-1.1 wt.%, Fe: 61.5-69.5 wt.%, the percentage refers to the mass percentage in the raw material composition of the RTB-based permanent magnet material.

In a preferred embodiment of the present invention, the raw material composition of the RTB-based permanent magnet material comprises the following components: R': 29.5-33.5 wt.%, Pr ≥ 8.85 wt.%, Cu: 0.34-0.51 wt.%, Al: 0-0.8 wt.%, but not 0, B: 0.95-1.1 wt.%, Fe: 61.5-69.5 wt.%, the percentage refers to the mass percentage in the raw material composition of the RTB-based permanent magnet material.

In a preferred embodiment of the present invention, the raw material composition of the RTB-based permanent magnet material comprises the following components: R': 29.5-33.5 wt.%, Pr > 8.85 wt.%, Cu: 0.34-0.51 wt.%, Al: 0-0.8 wt.%, but not 0, Ga: 0.1-0.5 wt.%, B: 0.95-1.1 wt.%, Fe: 61.5-69.5 wt.%, the percentage refers to the mass percentage in the raw material composition of the RTB-based permanent magnet material;

In a preferred embodiment of the present invention, the raw material composition of the RTB-based permanent magnet material comprises the following components: R': 29.5-33.5 wt.%, Pr ≥ 8.85 wt.%, Cu: 0.34-0.5 wt.%, Al: 0.3-0.8 wt.%, Ga: 0.1-0.4 wt.%, Zr: 0.25-0.30 wt.%, B: 0.95-1.1 wt.%, Fe: 61.5-69.5 wt.%, the percentage refers to the mass percentage in the raw material composition of the RTB-based permanent magnet material.

In the present invention, the molten liquid of the raw material composition of the RTB-based permanent magnet material is obtained by melting in a vacuum induction melting furnace. The vacuum degree of the melting furnace is 5×10⁻² Pa. The melting temperature is 1500°C or less.

In the present invention, the casting process is the conventional casting process in this field, with cooling at a rate of 10² °C /s to 10⁴°C/s in an Ar atmosphere.

In the present invention, the process of hydrogen decrepitation can be the conventional hydrogen decrepitation process in this field, for example, being subjected to hydrogen absorption, dehydrogenation and cooling treatment.

Wherein, the hydrogen absorption can be carried out at the hydrogen pressure of 0.15 MPa.

Wherein, the dehydrogenation can be carried out under the condition of both vacuum-pumping and heating.

In the present invention, the process of pulverization is jet mill pulverization.

The pressure in the pulverization chamber of the jet mill pulverization is 0.38 MPa.

The time of the jet mill pulverization is 3 hours.

In the present invention, preferably, during the pulverization process, the content of oxygen O in the pulverization atmosphere is 0-50 ppm, such as 0 ppm, 5 ppm, 10 ppm, 15 ppm, 20 ppm, 25 ppm, 30 ppm, 35 ppm, 40 ppm, 45 ppm, or 50 ppm.

In the present invention, the dispersant can be a dispersant routinely added in the preparation process of R-T-B-based permanent magnet materials, generally a lubricant and/or an antioxidant. Generally speaking, the lubricant and antioxidant added in the preparation of R-T-B-based magnet materials contain C element.

Wherein, the lubricant can be zinc stearate.

In the present invention, the amount of the dispersant is preferably 0.04-0.14%, such as 0.04%, 0.05%, 0.06%, 0.07%, 0.08%, 0.09%, 0.1%, 0.11%, 0.12%, 0.13% or 0.14%, the percentage refers to the mass percentage with respect to the total mass of the mixed powder.

When the dispersant contains zinc stearate, the amount of zinc stearate can be 0.04-0.14%, such as 0.04%, 0.05%, 0.06%, 0.07%, 0.08%, 0.09%, 0.1%, 0.11%, 0.12%, 0.13% or 0.14%, the percentage refers to the mass percentage with respect to the total mass of the mixed powder.

In the present invention, preferably, the content of oxygen O in the pressing atmosphere is 10-30 ppm, during the pressing process, such as 10 ppm, 12 PPM, 14 ppm, 16 ppm, 18 ppm, 20 ppm, 22 ppm, 24 ppm, 26 ppm, 28 ppm or 30 ppm.

In the present invention, the forming process can be a conventional forming process in this field, such as magnetic field forming method or hot pressing and hot deformation method.

In the present invention, the sintering process is the conventional sintering process in this field, for example, under the vacuum condition (for example, under the vacuum of 5 × 10⁻³Pa), being subjected to preheating, sintering, cooling.

Wherein, the temperature of the preheating can be 300-600°C. The time of the preheating can be 1-2h. Preferably, the preheating is preheating at 300°C and 600°C for 1h respectively.

Wherein, the temperature of the sintering is 1040-1090°C, such as 1050°C.

Wherein, the time of the sintering is 2h,

Wherein, the Ar can be introduced to make the air pressure reach 0. 1MPa before cooling.

In the present invention, preferably, the grain boundary diffusion treatment is also carried out after sintering and before the aging treatment.

Wherein, the grain boundary diffusion treatment can be treated according to the conventional process in this field, for example, attaching substance containing Tb and/or substance containing Dy to the surface of the RTB-based permanent magnet material by evaporating, coating or sputtering, then carrying out diffusion heat treatment.

The substance containing Tb may be Tb metal, a Tb-containing compound (for example, a Tb-containing fluoride) or an alloy.

The substance containing Dy may be Dy metal, a Dy-containing compound (for example, a Dy-containing fluoride) or an alloy.

The temperature of the diffusion heat treatment is preferably 800-900°C, such as 850°C.

The time of the diffusion heat treatment is preferably 12-48h, such as 24h.

In the present invention, the treatment temperature of the aging treatment is 500-650°C, for example 600-650°C, such as 630°C.

Wherein, in the aging treatment, the heating rate of heating to 500-650°C is 3-5 °C/min. The starting point for the heating can be room temperature.

Wherein, the treatment time of the aging treatment is 3h.

The present invention also provides an RTB-based permanent magnet material prepared by the above method.

The production method provides an application of the R-T-B-based permanent magnet material as an electronic components.

Wherein, the fields of the application can be automobile drive field, wind power field, servo motor and home appliance field (such as air conditioning).

In the present invention, the room temperature refers to 25°C±5°C.

In the present invention, Pr is praseodymium, Nd is neodymium, Cu is copper, B is boron, Fe is iron, Al is aluminum, Ga is gallium, Co is cobalt, Zr is zirconium, Ti is titanium, Nb is niobium, Zn is zinc, Dy is dysprody, Tb is terbium, Mn is manganese, Ni is nickel, Ag is silver, In is indium, Sn is tin, Bi is bismuth, V is vanadium, Cr is chromium, Ta is tantalum, W is tungsten, O is oxygen, C is carbon, and N is nitrogen.

On the basis of conforming to the common knowledge in this field, the above optimal conditions can be combined at will, so as to obtain better examples of the present invention.

The reagents and raw materials used in the present invention are commercially available.

The positive progressive effect of the present invention is as follows:
(1) The RTB-based permanent magnet material in the present invention can achieve the improvement of the performance of permanent magnet materials in the absence of heavy rare earth, and the RTB-based permanent magnet material has excellent magnetic properties, high coercivity, high remanence and good temperature stability.
(2) The preparation process of RTB-based permanent magnet material does not need to control the content of carbon elements introduced in the process, and under the condition of higher carbon content in the magnet, the magnet still maintains excellent performance.

### Brief description of the drawings

Fig.1 is the microstructure scanning photo of the RTB-based permanent magnet material prepared in embodiment 68, wherein, the position referred to by a is the intergranular triangle region.

### Detailed description of the preferred embodiment

The following examples further illustrate the present disclosure, but the present disclosure is not limited thereto. Experimental methods for which specific conditions are not specified in the following embodiments shall be selected in accordance with conventional methods and conditions, or in accordance with the commodity description. In the following table, wt.% refers to the percentage by mass of the component in the raw material composition of the RTB-based permanent magnet material, and "/" means that the element is not added. "Br" refers to remanence, and "Hcj" refers to intrinsic coercivity.

The formulas of RTB-based permanent magnet materials of the embodiments and comparative embodiments are shown in Table 1.

**Table 1**

| No. | R kind | R conte nt | Nd wt. % | Pr wt. % | RH kin d | RH wt. % | Cu wt. % | Al wt.% | Ga wt. % | Co wt. % | Zr wt. % | Nb wt. % | Mn wt. % | M kin d | M wt. % | B wt. % | Fe wt.% |
|---|---|---|---|---|---|---|---|---|---|---|---|---|---|---|---|---|---|
| Embodim ent 1 | / | / | 21.6 5 | 8.85 | / | / | / | / | / | / | / | / | / | / | / | 0.95 | remainder |
| Embodim ent 2 | / | / | 19.6 5 | 10.8 5 | / | / | / | / | / | / | / | / | / | / | / | 0.95 | remainder |
| Embodim ent 3 | / | / | 18.3 5 | 12.1 5 | / | / | / | / | / | / | / | / | / | / | / | 0.95 | remainder |
| Embodim ent 4 | / | / | 16.3 5 | 14.1 5 | / | / | / | / | / | / | / | / | / | / | / | 0.95 | remainder |
| Embodim ent 5 | / | / | 14.3 5 | 16.1 5 | / | / | / | / | / | / | / | / | / | / | / | 0.95 | remainder |
| Embodim ent 6 | / | / | 13.3 5 | 17.1 5 | / | / | / | / | / | / | / | / | / | / | / | 0.95 | remainder |
| Embodim ent 7 | / | / | 11.3 5 | 19.1 5 | / | / | / | / | / | / | / | / | / | / | / | 0.95 | remainder |
| Embodiment 8 | / | / | 9.35 | 21.15 | / | / | / | / | / | / | / | / | / | / | / | 0.95 | remainder |
| Embodim ent 9 | / | / | 7.35 | 23.1 5 | / | / | / | / | / | / | / | / | / | / | / | 0.95 | remainder |
| Embodim ent 10 | / | / | 5.35 | 25.1 5 | / | / | / | / | / | / | / | / | / | / | / | 0.95 | remainder |
| Embodim ent 11 | / | / | 3.35 | 27.1 5 | / | / | / | / | / | / | / | / | / | / | / | 0.95 | remainder |
| Embodim ent 12 | / | / | 22.1 5 | 8.85 | / | / | 0.20 | / | / | / | / | / | / | / | / | 0.95 | remainder |
| Embodim ent 13 | / | / | 18.8 5 | 12.1 5 | / | / | 0.30 | / | / | / | / | / | / | / | / | 1.01 | remainder |
| Embodim ent 14 | / | / | 13.8 5 | 17.1 5 | / | / | 0.35 | / | / | / | / | / | / | / | / | 1.01 | remainder |
| Embodim ent 15 | / | / | 10.8 5 | 20.1 5 | / | / | 0.45 | / | / | / | / | / | / | / | / | 1.01 | remainder |
| Embodim ent 16 | / | / | 7.85 | 23.1 5 | / | / | 0.50 | / | / | / | / | / | / | / | / | 1.01 | remainder |
| Embodim ent 17 | / | / | 22.1 5 | 8.85 | / | / | / | 0.02 | / | / | / | / | / | / | / | 1.01 | remainder |
| Embodim ent 18 | / | / | 20.8 5 | 10.1 5 | / | / | / | 0.04 2 | / | / | / | / | / | / | / | 0.95 | remainder |
| Embodim ent 19 | / | / | 18.8 5 | 12.1 5 | / | / | / | 0.1 | / | / | / | / | / | / | / | 0.95 | remainder |
| Embodim ent 20 | / | / | 16.8 5 | 14.1 5 | / | / | / | 0.2 | / | / | / | / | / | / | J | 0.95 | remainder |
| Embodim ent 21 | / | / | 14.8 5 | 16.1 5 | / | / | / | 0.3 | / | / | / | / | / | / | / | 0.95 | remainder |
| Embodim ent 22 | / | / | 13.8 5 | 17.1 5 | / | / | / | 0.4 | / | / | / | / | / | / | / | 0.95 | remainder |
| Embodim ent 23 | / | / | 11.8 5 | 19.1 5 | / | / | / | 0.5 | / | / | / | / | / | / | / | 0.95 | remainder |
| Embodim ent 24 | / | / | 10.8 5 | 20.1 5 | / | / | / | 0.6 | / | / | / | / | / | / | / | 0.95 | remainder |
| Embodim ent 25 | / | / | 8.85 | 22.1 5 | / | / | / | 0.7 | / | / | / | / | / | / | / | 0.95 | remainder |
| Embodim ent 26 | / | / | 6.85 | 24.1 5 | / | / | / | 0.8 | / | / | / | / | / | / | / | 0.95 | remainder |
| Embodim ent 27 | / | / | 20.6 5 | 8.85 | / | / | / | / | 0.1 | / | / | / | / | / | / | 0.95 | remainder |
| Embodim ent 28 | / | / | 19.6 8 | 9.85 | / | / | / | / | 0.2 | / | / | / | / | / | / | 0.98 | remainder |
| Embodim ent 29 | / | / | 18.6 5 | 10.8 5 | / | / | / | / | 0.25 | / | / | / | / | / | / | 0.98 | remainder |
| Embodim ent 30 | / | / | 17.6 5 | 11.8 5 | / | / | / | / | 0.30 | / | / | / | / | / | / | 0.98 | remainder |
| Embodim ent 31 | / | / | 17.3 5 | 12.1 5 | / | / | / | / | 0.42 | / | / | / | / | / | / | 0.98 | remainder |
| Embodim ent 32 | / | / | 16.3 5 | 13.1 5 | / | / | / | / | 0.50 | / | / | / | / | / | / | 0.98 | remainder |
| Embodim ent 33 | / | / | 15.3 5 | 14.1 5 | / | / | / | / | 0.90 | / | / | / | / | / | / | 0.98 | remainder |
| Embodim ent 34 | / | / | 9.35 | 20.1 5 | / | / | / | / | 1.40 | / | / | / | / | / | / | 0.98 | remainder |
| Embodim ent 35 | / | / | 8.35 | 21.1 5 | / | / | / | / | 1.55 | / | / | / | 0.01 | / | / | 0.98 | remainder |
| Embodim ent 36 | / | / | 14.3 5 | 175 | / | / | / | / | / | 0.5 | / | / | / | / | / | 0.98 | remainder |
| Embodim ent 37 | / | / | 13.3 5 | 18.1 5 | / | / | / | / | / | 1 | / | / | / | / | / | 0.98 | remainder |
| Embodim ent 38 | / | / | 12.3 5 | 19.1 5 | / | / | / | / | / | 2.5 | / | / | / | / | / | 1.01 | remainder |
| Embodim ent 39 | / | / | 14.3 5 | 17.1 5 | / | / | / | / | / | / | 0.25 | / | / | / | / | 1.01 | remainder |
| Embodim ent 40 | / | / | 13.3 5 | 18.1 5 | / | / | | | | / | 0.30 | / | / | / | / | 1.01 | remainder |
| Embodim ent 41 | / | / | 12.3 5 | 19.1 5 | / | / | / | / | / | / | 0.35 | / | / | / | / | 1.01 | remainder |
| Embodim ent 42 | / | / | 14.3 5 | 17.1 5 | / | / | / | / | / | / | / | 0.25 | / | / | / | 1.01 | remainder |
| Embodim ent 43 | / | / | 13.3 5 | 18.1 5 | / | / | / | / | / | / | / | 0.30 | / | / | / | 1.01 | remainder |
| Embodim ent 44 | / | / | 12.3 5 | 19.1 5 | / | / | / | / | / | / | / | 0.35 | / | / | / | 1.01 | remainder |
| Embodim ent 45 | / | / | 22.6 5 | 8.85 | / | / | 0.34 | 0.02 | / | / | / | / | / | / | / | 1.01 | remainder |
| Embodim ent 46 | / | / | 21.3 5 | 10.1 5 | / | / | 0.38 | 0.04 2 | / | / | / | / | / | / | / | 1.01 | remainder |
| Embodim ent 47 | / | / | 19.3 5 | 12.1 5 | / | / | 0.42 | 0.1 | / | / | / | / | / | / | / | 1.01 | remainder |
| Embodim ent 48 | / | / | 17.3 5 | 14.1 5 | / | / | 0.44 | 0.2 | / | / | / | / | / | / | / | 1.01 | remainder |
| Embodim ent 49 | / | / | 15.3 5 | 16.1 5 | / | / | 0.50 | 0.3 | / | / | / | / | / | / | / | 1.01 | remainder |
| Embodim ent 50 | / | / | 14.3 5 | 17.1 5 | / | / | 0.34 | 0.4 | / | / | / | / | / | / | / | 1.01 | remainder |
| Embodim ent 51 | / | / | 12.3 5 | 19.1 5 | / | / | 0.35 | 0.5 | / | / | / | / | / | / | / | 1.01 | remainder |
| Embodim ent 52 | / | / | 11.3 5 | 20.1 5 | / | / | 0.42 | 0.6 | / | / | / | / | / | / | / | 1.01 | remainder |
| Embodim ent 53 | / | / | 9.35 | 22.1 5 | / | / | 0.34 | 0.5 | 0.1 | / | / | / | / | / | / | 1.01 | remainder |
| Embodim ent 54 | / | / | 7.35 | 24.1 5 | / | / | 0.40 | 0.6 | 0.3 | / | / | / | / | / | / | 1.01 | remainder |
| Embodim ent 55 | / | / | 13.6 5 | 17.1 5 | / | / | 0.50 | 0.8 | 0.42 | / | / | / | / | / | / | 1.01 | remainder |
| Embodim ent 56 | / | / | 8.65 | 22.1 5 | / | / | 0.34 | 0.5 | 0.1 | / | 0.25 | / | / | / | / | 1.01 | remainder |
| Embodim ent 57 | / | / | 6.65 | 24.1 5 | / | / | 0.50 | 0.8 | 0.3 | / | 0.30 | / | / | / | / | 1.01 | remainder |
| Embodim ent 58 | / | / | 21.9 8 | 8.85 | / | / | 0.34 | 0.01 | 0.25 | / | / | / | / | / | / | 1.01 | remainder |
| Embodim ent 59 | / | / | 20.6 5 | 10.1 5 | / | / | 0.38 | 0.02 | 0.30 | / | / | / | / | / | / | 0.96 | Remainde r |
| Embodim ent 60 | / | / | 18.6 5 | 12.1 5 | / | / | 0.42 | 0.03 | 0.42 | / | / | / | / | / | / | 0.96 | remainder |
| Embodim ent 61 | / | / | 16.6 5 | 14.1 5 | / | / | 0.38 | 0.04 2 | 0.1 | / | / | / | / | / | / | 0.96 | remainder |
| Embodim ent 62 | / | / | 14.6 5 | 16.1 5 | / | / | 0.42 | 0.1 | 0.15 | / | / | / | / | / | / | 0.96 | remainder |
| Embodim ent 63 | / | / | 13.6 5 | 17.1 5 | / | / | 0.44 | 0.2 | 0.25 | / | / | / | / | / | / | 0.96 | remainder |
| Embodim ent 64 | / | / | 11.6 5 | 19.1 5 | / | / | 0.50 | 0.3 | 0.30 | / | / | / | / | / | / | 0.96 | remainder |
| Embodim ent 65 | / | / | 10.6 5 | 20.1 5 | / | / | 0.45 | 0.4 | 0.42 | / | / | / | / | / | / | 0.96 | remainder |
| Embodim ent 66 | / | / | 8.65 | 22.1 5 | / | / | 0.50 | 0.5 | 0.50 | / | / | / | / | / | / | 1.01 | remainder |
| Embodim ent 67 | / | / | 12.6 5 | 18.1 5 | / | / | 0.4 | 0.6 | 0.4 | 2.5 | 0.3 | / | / | Cr | 0.05 | 1.01 | remainder |
| Embodim ent 68 | / | / | 12.6 5 | 18.1 5 | / | / | 0.4 | 0.6 | 0.4 | 2.5 | 0.3 | / | / | Cr | 0.12 | 1.01 | remainder |
| Embodim ent 69 | / | / | 13.6 5 | 17.1 5 | Dy | 1.5 | 0.4 | 0.3 | 0.30 | 2.5 | 0.3 | / | / | / | / | 1.01 | remainder |
| Embodim ent 70 | / | / | 12.6 5 | 18.1 5 | Dy | 2.0 | 0.4 | 0.3 | 0.30 | 2.5 | 0.3 | / | / | / | / | 0.96 | remainder |
| Embodim ent 71 | / | / | 11.6 5 | 19.1 5 | Dy | 2.5 | 0.4 | 0.35 | 0.30 | 2.5 | 0.3 | / | / | / | / | 0.96 | remainder |
| Embodim ent 72 | / | / | 11.6 5 | 19.1 5 | Dy | 2.5 | 0.4 | 0.45 | 0.30 | 2.5 | 0.3 | / | / | / | / | 0.96 | remainder |
| Embodim ent 73 | / | / | 13.6 5 | 17.1 5 | Tb | 2 | 0.4 | 0.3 | 0.30 | 2.5 | 0.3 | / | / | / | / | 0.96 | remainder |
| Embodim ent 74 | / | / | 12.6 5 | 18.1 5 | Tb | 1.2 | 0.4 | 0.3 | 0.30 | 2.5 | 0.3 | / | / | / | / | 0.96 | remainder |
| Embodim ent 75 | Ce | 0.3 | 11.3 5 | 18.1 5 | Tb | 1.2 | 0.4 | 0.6 | 0.4 | 2.5 | 0.3 | / | / | / | / | 0.96 | remainder |
| Comparat ive Embodim ent 1 | / | / | 22 | 8.00 | / | / | / | / | / | / | / | / | / | / | / | 0.96 | remainder |
| Comparat ive Embodim ent 2 | / | / | 22 | 8.00 | / | / | 0.4 | 0 | 0.4 | 2.5 | 0.3 | / | / | Cr | 0.12 | 0.96 | remainder |

### Embodiment 1

The preparation method for the RTB-based permanent magnet material is as follows:
(1) Melting process: according to the formula shown in Table 1, the pre-made raw materials were put into the crucible made of aluminum oxide, and was vacuum melted in the high frequency vacuum induction melting furnace and in a vacuum of 5×10⁻²Pa at a temperature of 1500°C or less.
(2) Casting process: Ar gas was introduced into the melting furnace after vacuum melting to make the air pressure reach 55,000 Pa, and then casting was carried out, and quenching alloy was obtained at the cooling rate of 10² °C/s to 10⁴ °C/s.
(3) Hydrogen decrepitation process: the hydrogen decrepitation furnace with quench alloy placed therein was vacuumed at room temperature, and then hydrogen with a purity of 99.9% was introduced into the hydrogen decrepitation furnace to maintain the hydrogen pressure at 0.15MPa; after full hydrogen absorption, the temperature was raised while vacuuming for full dehydrogenation; then cooled, and took out the powder obtained from hydrogen decrepitation.
(4) Micro-pulverization process: In nitrogen atmosphere and under the condition of a pressure of 0.38MPa in the pulverization chamber, the powder obtained from hydrogen decrepitation was pulverized by jet mill pulverization for 3 hours to obtain fine powder. The content of oxygen (ppm) in nitrogen atmosphere is shown in Table 2.
(5) The zinc stearate was added to the powder obtained from jet mill pulverization, and mixed fully by v-type mixer. The added amount of zinc stearate is shown in Table 2, and the percentage refers to the weight percentage in the mixed powder.
(6) Magnetic field forming process: The rectangular oriented magnetic field forming machine was used to form the above powder with zinc stearate into a cube with sides of 25mm in a oriented magnetic field of 1.6T and under the molding pressure of 0.35ton/cm²; demagnetization was carried out in a magnetic field of 0.2T after forming. The content of O (oxygen) in the atmosphere during the pressing process was shown in Table 2. In order to prevent the formed body after the first forming from contacting the air, it was sealed, and then the secondary forming was carried out with the secondary forming machine (isostatic pressing machine) under the pressure of 1.3ton/cm².
(7) Sintering process: each formed body was moved to the sintering furnace for sintering, sintered in the vacuum of 5×10⁻³Pa and at 300°C and 600°C for 1 hour respectively; then, it was sintered at the temperature of 1050°C for 2 hours; Ar was then introduced to make the air pressure reach 0.1MPa and then cooled to room temperature.
(8) Aging treatment process: The sintered body was heated from 20°C to 630°C at a heating rate of 3-5°C /min in the Ar of high purity; after 3 hours of heat treatment at 630°C, it was cooled to room temperature and taken out.

### Embodiments 2-75, Comparative Embodiments 1-2

The formulas of Embodiments 2-75, comparative embodiments 1-2 are shown in Table 1, the preparation process is shown in Table 2, and the remaining steps are the same as those in Embodiment 1.

### Embodiment 76

The sintered body obtained in Embodiment 1 was first subjected to grain boundary diffusion treatment and then to aging treatment. The preparation process is shown in Table 2, and the other steps are the same as those in Embodiment 1. The process of grain boundary diffusion treatment is as follows:
The sintered body was processed into the magnet with diameter of 20 mm, and the thickness of the sheet material was less than 7 mm, the direction of the thickness was the direction of magnetic field orientation, after the surface was cleaned, the raw material prepared with Dy fluoride was coated on the magnet through fully spraying respectively, after drying the coated magnet, the metal attached with Dy was sputtered on the surface of the magnet in the high purity Ar atmosphere, and diffusing heat treatment was carried out at 850°C for 24 hours. Cooled to room temperature.

### Embodiment 77

The sintered body obtained in Embodiment 1 was first subjected to grain boundary diffusion treatment and then to aging treatment. The preparation process is shown in Table 2, and the other steps are the same as those in Embodiment 1. The process of grain boundary diffusion treatment is as follows:
The sintered body was processed into the magnet with diameter of 20 mm, and the thickness of the sheet material was less than 7 mm, the direction of the thickness was the direction of magnetic field orientation, after the surface was cleaned, the raw material prepared with Tb fluoride was coated on the magnet through fully spraying respectively, after drying the coated magnet, the metal attached with Tb was sputtered on the surface of the magnet in the high purity Ar atmosphere, and diffusing heat treatment was carried out at 850°C for 24 hours. Cooled to room temperature.

**Table 2**

| No. | Content of O (ppm) in the milling process of step 4 | Amount of zinc stearate (%) added in Step 5 | Content of O (ppm) in the pressing process of step 6 | Grain boundary diffusion (Y/N) | Elements in grain boundary diffusion |
|---|---|---|---|---|---|
| Embodiment 1 | 0 | 0.04 | 10 | N | / |
| Embodiment 2 | 5 | 0.05 | 12 | N | / |
| Embodiment 3 | 10 | 0.06 | 14 | N | / |
| Embodiment 4 | 15 | 0.07 | 16 | N | / |
| Embodiment 5 | 20 | 0.08 | 18 | N | / |
| Embodiment 6 | 25 | 0.09 | 20 | N | / |
| Embodiment 7 | 30 | 0.10 | 22 | N | / |
| Embodiment 8 | 35 | 0.11 | 24 | N | / |
| Embodiment 9 | 40 | 0.12 | 26 | N | / |
| Embodiment 10 | 45 | 0.13 | 28 | N | / |
| Embodiment 11 | 50 | 0.14 | 30 | N | / |
| Embodiment 12 | 0 | 0.04 | 10 | N | / |
| Embodiment 13 | 5 | 0.05 | 12 | N | / |
| Embodiment 14 | 10 | 0.06 | 14 | N | / |
| Embodiment 15 | 15 | 0.07 | 16 | N | / |
| Embodiment 16 | 20 | 0.08 | 18 | N | / |
| Embodiment 17 | 25 | 0.09 | 20 | N | / |
| Embodiment 18 | 30 | 0.10 | 22 | N | / |
| Embodiment 19 | 35 | 0.11 | 24 | N | / |
| Embodiment 20 | 40 | 0.12 | 26 | N | / |
| Embodiment 21 | 45 | 0.13 | 28 | N | / |
| Embodiment 22 | 50 | 0.14 | 30 | N | / |
| Embodiment 23 | 15 | 0.07 | 16 | N | / |
| Embodiment 24 | 20 | 0.08 | 18 | N | / |
| Embodiment 25 | 15 | 0.07 | 16 | N | / |
| Embodiment 26 | 20 | 0.08 | 18 | N | / |
| Embodiment 27 | 0 | 0.04 | 10 | N | / |
| Embodiment 28 | 5 | 0.05 | 12 | N | / |
| Embodiment 29 | 10 | 0.06 | 14 | N | / |
| Embodiment 30 | 15 | 0.07 | 16 | N | / |
| Embodiment 31 | 20 | 0.08 | 18 | N | / |
| Embodiment 32 | 25 | 0.09 | 20 | N | / |
| Embodiment 33 | 30 | 0.10 | 22 | N | / |
| Embodiment 34 | 35 | 0.11 | 24 | N | / |
| Embodiment 35 | 40 | 0.12 | 26 | N | / |
| Embodiment 36 | 0 | 0.04 | 10 | N | / |
| Embodiment 37 | 5 | 0.05 | 12 | N | / |
| Embodiment 38 | 10 | 0.06 | 14 | N | / |
| Embodiment 39 | 15 | 0.07 | 16 | N | / |
| Embodiment 40 | 20 | 0.08 | 18 | N | / |
| Embodiment 41 | 25 | 0.09 | 20 | N | / |
| Embodiment 42 | 30 | 0.10 | 22 | N | / |
| Embodiment 43 | 35 | 0.11 | 24 | N | / |
| Embodiment 44 | 40 | 0.12 | 26 | N | / |
| Embodiment 45 | 45 | 0.13 | 28 | N | / |
| Embodiment 46 | 50 | 0.14 | 30 | N | / |
| Embodiment 47 | 15 | 0.07 | 16 | N | / |
| Embodiment 48 | 20 | 0.08 | 18 | N | / |
| Embodiment 49 | 15 | 0.07 | 16 | N | / |
| Embodiment 50 | 20 | 0.08 | 18 | N | / |
| Embodiment 51 | 15 | 0.07 | 16 | N | / |
| Embodiment 52 | 20 | 0.08 | 18 | N | / |
| Embodiment 53 | 15 | 0.07 | 16 | N | / |
| Embodiment 54 | 20 | 0.08 | 18 | N | / |
| Embodiment 55 | 0 | 0.04 | 10 | N | / |
| Embodiment 56 | 5 | 0.05 | 12 | N | / |
| Embodiment 57 | 10 | 0.06 | 14 | N | / |
| Embodiment 58 | 15 | 0.07 | 16 | N | / |
| Embodiment 59 | 20 | 0.08 | 18 | | |
| Embodiment 60 | 25 | 0.09 | 20 | | |
| Embodiment 61 | 30 | 0.10 | 22 | N | / |
| Embodiment 62 | 35 | 0.11 | 24 | N | / |
| Embodiment 63 | 40 | 0.12 | 26 | N | / |
| Embodiment 64 | 45 | 0.13 | 28 | N | / |
| Embodiment 65 | 50 | 0.14 | 30 | N | / |
| Embodiment 66 | 15 | 0.07 | 16 | N | / |
| Embodiment 67 | 0 | 0.04 | 10 | N | / |
| Embodiment 68 | 5 | 0.05 | 12 | N | / |
| Embodiment 69 | 10 | 0.06 | 14 | N | / |
| Embodiment 70 | 15 | 0.07 | 16 | N | / |
| Embodiment 71 | 20 | 0.08 | 18 | N | / |
| Embodiment 72 | 25 | 0.09 | 20 | N | / |
| Embodiment 73 | 30 | 0.10 | 22 | N | / |
| Embodiment 74 | 35 | 0.11 | 24 | N | / |
| Embodiment 75 | 40 | 0.12 | 26 | N | / |
| Embodiment 76 | 0 | 0.04 | 10 | Y | Dy |
| Embodiment 77 | 0 | 0.04 | 10 | Y | Tb |
| Comparative Embodiment 1 | 20 | 0.08 | 18 | N | / |
| Comparative Embodiment 2 | 20 | 0.08 | 18 | N | / |

| | | | | | |
|---|---|---|---|---|---|
| Note: The percentage of zinc stearate added refers to the weight percentage in the mixed powder, and the content of O (oxygen) refers to the content of O (oxygen) atom in the atmosphere. | | | | | |

### Effect embodiment

The magnetic properties and composition of RTB-based permanent magnet materials prepared in Embodiments 1-77 and Comparative embodiments 1-2 were determined, and the crystal phase structure of the magnets was observed by Fe-EPMA.
(1) Evaluation of magnetic properties: The NIM-10000H BH bulk rare earth permanent magnetic nondestructive measurement system in National Institute of Metrology, China was used for magnetic properties detection of permanent magnetic materials. The test results of magnetic properties are shown in Table 3 below, wherein 1 kGs = 0.1 T and 1 kOe = 79.6 kA/m.

**Table 3**

| No. | Br(kGs) | Hcj(kOe) | Absolute value of Hcj temperature coefficient at 80 °C | Absolute value of Hcj temperature coefficient at 150 °C | Absolute value of Hcj temperature coefficient at 180 °C |
|---|---|---|---|---|---|
| Embodiment 1 | 14.5 | 16.37 | 0.748 | / | / |
| Embodiment 2 | 14.51 | 16.9 | 0.735 | / | / |
| Embodiment 3 | 14.48 | 17.23 | 0.701 | / | / |
| Embodiment 4 | 14.42 | 17.75 | 0.662 | / | / |
| Embodiment 5 | 14.37 | 18.26 | 0.647 | / | / |
| Embodiment 6 | 14.35 | 18.51 | 0.653 | / | / |
| Embodiment 7 | 14.30 | 19.03 | 0.648 | / | / |
| Embodiment 8 | 14.25 | 19.54 | 0.642 | / | / |
| Embodiment 9 | 14.2 | 20.05 | 0.637 | / | / |
| Embodiment 10 | 14.15 | 20.56 | 0.631 | / | / |
| Embodiment 11 | 14.11 | 21.08 | 0.626 | / | / |
| Embodiment 12 | 14.34 | 17.06 | 0.715 | / | / |
| Embodiment 13 | 14.16 | 18.14 | 0.652 | / | / |
| Embodiment 14 | 14.03 | 19.54 | 0.641 | / | / |
| Embodiment 15 | 13.91 | 20.55 | 0.632 | / | / |
| Embodiment 16 | 13.82 | 21.32 | 0.622 | / | / |
| Embodiment 17 | 14.32 | 16.68 | 0.731 | / | / |
| Embodiment 18 | 14.27 | 17.12 | 0.715 | / | / |
| Embodiment 19 | 14.17 | 17.92 | 0.668 | / | / |
| Embodiment 20 | 14.02 | 18.93 | 0.648 | / | / |
| Embodiment 21 | 13.88 | 19.94 | 0.639 | / | / |
| Embodiment 22 | 13.76 | 20.7 | 0.637 | / | / |
| Embodiment 23 | 13.62 | 21.71 | 0.618 | / | / |
| Embodiment 24 | 13.5 | 22.46 | 0.605 | / | / |
| Embodiment 25 | 13.36 | 23.47 | 0.597 | / | / |
| Embodiment 26 | 13.22 | 24.48 | / | / | / |
| Embodiment 27 | 14.68 | 16.58 | 0.734 | 0.524 | / |
| Embodiment 28 | 14.65 | 17.51 | 0.668 | / | / |
| Embodiment 29 | 14.61 | 18.11 | 0.653 | / | / |
| Embodiment 30 | 14.55 | 18.70 | 0.651 | / | / |
| Embodiment 31 | 14.43 | 19.59 | 0.641 | / | / |
| Embodiment 32 | 14.38 | 20.39 | 0.636 | / | / |
| Embodiment 33 | 14.3 | 22.85 | 0.601 | 0.526 | / |
| Embodiment 34 | 13.95 | 24.39 | / | 0.522 | / |
| Embodiment 35 | 13.93 | 24.42 | / | / | / |
| Embodiment 36 | 14.02 | 18.43 | 0.668 | / | / |
| Embodiment 37 | 14.39 | 18.69 | 0.654 | / | / |
| Embodiment 38 | 13.72 | 19.45 | 0.648 | / | / |
| Embodiment 39 | 13.85 | 18.61 | 0.657 | / | / |
| Embodiment 40 | 13.81 | 18.81 | 0.653 | / | / |
| Embodiment 41 | 13.76 | 19.19 | 0.649 | / | / |
| Embodiment 42 | 13.89 | 18.59 | 0.656 | / | / |
| Embodiment 43 | 13.86 | 18.75 | 0.652 | / | / |
| Embodiment 44 | 13.80 | 19.08 | 0.651 | / | / |
| Embodiment 45 | 14.09 | 17.22 | 0.713 | / | / |
| Embodiment 46 | 14.05 | 17.76 | 0.710 | / | / |
| Embodiment 47 | 13.94 | 18.65 | 0.654 | / | / |
| Embodiment 48 | 13.81 | 19.71 | 0.639 | / | / |
| Embodiment 49 | 13.58 | 20.86 | 0.637 | / | / |
| Embodiment 50 | 13.54 | 21.23 | 0.621 | / | / |
| Embodiment 51 | 13.38 | 22.34 | 0.610 | / | / |
| Embodiment 52 | 13.25 | 23.19 | 0.602 | / | / |
| Embodiment 53 | 13.33 | 23.69 | 0.594 | / | / |
| Embodiment 54 | 13.02 | 24.49 | / | 0.523 | / |
| Embodiment 55 | 13.05 | 24.43 | / | 0.521 | / |
| Embodiment 56 | 13.49 | 21.67 | 0.618 | / | / |
| Embodiment 57 | 12.95 | 25.41 | / | 0.515 | / |
| Embodiment 58 | 14.17 | 16.97 | 0.735 | / | / |
| Embodiment 59 | 14.24 | 17.66 | 0.713 | / | / |
| Embodiment 60 | 13.9 | 19.13 | 0.651 | / | / |
| Embodiment 61 | 14.12 | 17.44 | 0.672 | / | / |
| Embodiment 62 | 13.92 | 18.68 | 0.652 | / | / |
| Embodiment 63 | 13.7 | 20.15 | 0.639 | / | / |
| Embodiment 64 | 13.56 | 21.64 | 0.619 | / | / |
| Embodiment 65 | 13.41 | 23.09 | 0.605 | / | / |
| Embodiment 66 | 13.3 | 24.76 | / | 0.519 | / |
| Embodiment 67 | 13.15 | 24.02 | / | 0.521 | / |
| Embodiment 68 | 13.12 | 24.21 | / | 0.519 | / |
| Embodiment 69 | 12.39 | 27.81 | / | 0.491 | / |
| Embodiment 70 | 12.31 | 29.42 | / | 0.488 | / |
| Embodiment 71 | 11.95 | 31.02 | / | / | 0.442 |
| Embodiment 72 | 12.01 | 30.51 | / | / | 0.448 |
| Embodiment 73 | 12.11 | 31.09 | / | / | 0.442 |
| Embodiment 74 | 12.39 | 29.39 | / | 0.488 | / |
| Embodiment 75 | 12.35 | 23.03 | 0.605 | / | / |
| Embodiment 76 | 14.32 | 22.38 | 0.610 | / | / |
| Embodiment 77 | 14.35 | 28.15 | / | 0.503 | / |
| Comparative Embodiment 1 | 13.8 | 14.9 | 0.803 | / | / |
| Comparative Embodiment 2 | 14.1 | 14.2 | 0.819 | / | / |

(2) Composition determination: The components were determined by high frequency inductively coupled plasma emission spectrometer (ICP-OES). The composition test results are shown in Table 4 below.

**Table 4**

| No. | R kind | R dose | Nd wt.% | Pr wt.% | RH kind | RH wt.% | Cu wt.% | Al wt.% | Ga wt.% | Co wt.% | Zr wt.% | Nb wt.% | Mn wt.% | M kind | M wt.% | B wt.% | Fe wt.% | C wt.% | O wt.% | N wt.% |
|---|---|---|---|---|---|---|---|---|---|---|---|---|---|---|---|---|---|---|---|---|
| Embodim ent 1 | / | / | 21.648 | 8.849 | / | / | / | / | / | / | / | / | / | / | / | 0.948 | remainder | 0.1069 | 0.039 | 0.0482 |
| Embodim ent 2 | / | / | 19.649 | 10.849 | / | / | / | / | / | / | / | / | / | / | / | 0.947 | remainder | 0.1251 | 0.0412 | 0.0458 |
| Embodim ent 3 | / | / | 18.335 | 12.151 | / | / | / | / | / | / | / | / | / | / | / | 0.951 | remainder | 0.1532 | 0.0432 | 0.0439 |
| Embodim ent 4 | / | / | 16.349 | 14.152 | / | / | / | / | / | / | / | / | / | / | / | 0.952 | remainder | 0.1759 | 0.0468 | 0.0401 |
| Embodim ent 5 | / | / | 14.348 | 16.151 | / | / | / | / | / | / | / | / | / | / | / | 0.951 | remainder | 0.1835 | 0.0493 | 0.0375 |
| Embodim ent 6 | / | / | 13.348 | 17.152 | / | / | / | / | / | / | / | / | / | / | / | 0.947 | remainder | 0.1965 | 0.0523 | 0.0342 |
| Embodim ent 7 | / | / | 11.3481 | 19.15 | / | / | / | / | / | / | / | / | / | / | / | 0.951 | remainder | 0.2139 | 0.0558 | 0.0302 |
| Embodim ent 8 | / | / | 9.349 | 21.148 | / | / | / | / | / | / | / | / | / | / | / | 0.947 | remainder | 0.2248 | 0.0635 | 0.0251 |
| Embodim ent 9 | / | / | 7.351 | 23.149 | / | / | / | / | / | / | / | / | / | / | / | 0.947 | remainder | 0.2248 | 0.0635 | 0.0251 |
| Embodim ent 10 | / | / | 5.352 | 25.152 | / | / | / | / | / | / | / | / | / | / | / | 0.951 | remainder | 0.2379 | 0.0669 | 0.0223 |
| Embodim ent 11 | / | / | 3.348 | 27.148 | / | / | / | / | / | / | / | / | / | / | / | 0.947 | remainder | 0.2456 | 0.0685 | 0.0182 |
| Embodim ent 12 | / | / | 22.149 | 8.851 | / | / | 0.201 | / | / | / | / | / | / | / | / | 0.951 | remainder | 0.1072 | 0.0382 | 0.0482 |
| Embodim ent 13 | / | / | 18.849 | 12.15 | / | / | 0.302 | / | / | / | / | / | / | / | / | 1.011 | remainder | 0.1256 | 0.0442 | 0.0461 |
| Embodim ent 14 | / | / | 13.848 | 17.15 | / | / | 0.351 | / | / | / | / | / | / | / | / | 1.009 | remainder | 0.1537 | 0.0456 | 0.0442 |
| Embodim ent 15 | / | / | 10.851 | 20.15 | / | / | 0.451 | / | / | / | / | / | / | / | / | 1.008 | remainder | 0.1764 | 0.0492 | 0.0404 |
| Embodim ent 16 | / | / | 7.849 | 23.15 | / | / | 0.50 | / | / | / | / | / | / | / | / | 0.998 | remainder | 0.1843 | 0.0501 | 0.0378 |
| Embodim ent 17 | / | / | 22.149 | 8.848 | / | / | / | 0.021 | / | / | / | / | / | / | / | 1.011 | remainder | 0.1973 | 0.0529 | 0.0347 |
| Embodim ent 18 | / | / | 20.851 | 10.151 | / | / | / | 0.041 | / | / | / | / | / | / | / | 0.949 | remainder | 0.2147 | 0.0564 | 0.0307 |
| Embodim ent 19 | / | / | 18.849 | 12.148 | / | / | / | 0.101 | / | / | / | / | / | / | / | 0.948 | remainder | 0.2251 | 0.0588 | 0.029 |
| Embodim ent 20 | / | / | 16.848 | 14.149 | / | / | / | 0.202 | / | / | / | / | / | / | / | 0.948 | remainder | 0.2248 | 0.0641 | 0.0256 |
| Embodim ent 21 | / | / | 14.849 | 16.151 | / | / | / | 0.301 | / | / | / | / | / | / | / | 0.949 | remainder | 0.2379 | 0.0675 | 0.0228 |
| Embodim ent 22 | / | / | 13.852 | 17.151 | / | / | / | 0.401 | / | / | / | / | / | / | / | 0.949 | remainder | 0.2456 | 0.0691 | 0.0187 |
| Embodim ent 23 | / | / | 11.851 | 19.150 | / | / | / | 0.497 | / | / | / | / | / | / | / | 0.948 | remainder | 0.1761 | 0.0494 | 0.0397 |
| Embodim ent 24 | / | / | 10.851 | 20.152 | / | / | / | 0.602 | / | / | / | / | / | / | / | 0.951 | remainder | 0.184 | 0.0503 | 0.0371 |
| Embodim ent 25 | / | / | 8.852 | 22.151 | / | / | / | 0.702 | / | / | / | / | / | / | / | 0.949 | remainder | 0.1761 | 0.0494 | 0.0397 |
| Embodim ent 26 | / | / | 6.851 | 24.152 | / | / | / | 0.801 | / | / | / | / | / | / | / | 0.95 | remainder | 0.1846 | 0.05 | 0.0366 |
| Embodim ent 27 | / | / | 20.652 | 8.851 | / | / | / | / | 0.102 | / | / | / | / | / | / | 0.948 | remainder | 0.1069 | 0.0384 | 0.0476 |
| Embodim ent 28 | / | / | 19.652 | 9.85 | / | / | / | / | 0.2 | / | / | / | / | / | / | 0.981 | remainder | 0.1253 | 0.0444 | 0.0455 |
| Embodim ent 29 | / | / | 18.651 | 10.848 | / | / | / | / | 0.251 | / | / | / | / | / | / | 0.982 | remainder | 0.1534 | 0.0458 | 0.0436 |
| Embodim ent 30 | / | / | 17.652 | 11.848 | / | / | / | / | 0.302 | / | / | / | / | / | / | 0.985 | remainder | 0.1761 | 0.0494 | 0.0398 |
| Embodim ent 31 | / | / | 17.352 | 12.148 | / | / | / | / | 0.421 | / | / | / | / | / | / | 0.981 | remainder | 0.184 | 0.0503 | 0.0341 |
| Embodim ent 32 | / | / | 16.350 | 13.149 | / | / | / | / | 0.501 | / | / | / | / | / | / | 0.982 | remainder | 0.197 | 0.0531 | 0.0341 |
| Embodim ent 33 | / | / | 15.353 | 14.148 | / | / | / | / | 0.901 | / | / | / | / | / | / | 0.985 | remainder | 0.2144 | 0.0566 | 0.0301 |
| Embodim ent 34 | / | / | 9.352 | 20.148 | / | / | / | / | 1.402 | / | / | / | / | / | / | 0.981 | remainder | 0.2248 | 0.059 | 0.0284 |
| Embodim ent 35 | / | / | 8.351 | 21.148 | / | / | / | / | 1.552 | / | / | / | 0.01 | / | / | 0.982 | remainder | 0.2245 | 0.0643 | 0.025 |
| Embodim ent 36 | / | / | 14.335 | 17.149 | / | / | / | / | / | 0.501 | / | / | / | / | / | 0.985 | remainder | 0.1759 | 0.0468 | 0.0401 |
| Embodim ent 37 | / | / | 13.352 | 18.148 | / | / | / | / | / | 1.021 | / | / | / | / | / | 0.981 | remainder | 0.1835 | 0.0493 | 0.0375 |
| Embodim ent 38 | / | / | 12.352 | 19.148 | / | / | / | / | / | 2.501 | / | / | / | / | / | 1.010 | remainder | 0.1965 | 0.0523 | 0.0342 |
| Embodim ent 39 | / | / | 14.351 | 17.148 | / | / | / | / | / | / | 0.251 | / | / | / | / | 1.009 | remainder | 0.2139 | 0.0558 | 0.0302 |
| Embodim ent 40 | / | / | 13.352 | 18.149 | / | / | / | / | / | / | 0.301 | / | / | / | / | 1.011 | remainder | 0.2243 | 0.0582 | 0.0285 |
| Embodim ent 41 | / | / | 12.351 | 19.149 | / | / | / | / | / | / | 0.351 | / | / | / | / | 1.010 | remainder | 0.1072 | 0.0382 | 0.0482 |
| Embodim ent 42 | / | / | 14.35 | 17.148 | / | / | / | / | / | / | / | 0.25 1 | / | / | / | 1.009 | remainder | 0.2379 | 0.0669 | 0.0223 |
| Embodim ent 43 | / | / | 13.353 | 18.151 | / | / | / | / | / | / | / | 0.30 1 | / | / | / | 1.001 1 | remainder | 0.2456 | 0.0685 | 0.0182 |
| Embodim ent 44 | / | / | 12.351 | 19.148 | / | / | / | / | / | / | / | 0.35 1 | / | / | / | 1.010 | remainder | 0.1072 | 0.0382 | 0.0482 |
| Embodim ent 45 | / | / | 22.652 | 8.848 | / | / | 0.341 | 0.021 | / | / | / | / | / | / | / | 1.009 | remainder | 0.1256 | 0.0442 | 0.0461 |
| Embodim ent 46 | / | / | 21.353 | 10.149 | / | / | 0.382 | 0.041 | / | / | / | / | / | / | / | 1.010 | remainder | 0.1537 | 0.0456 | 0.0442 |
| Embodim ent 47 | / | / | 19.351 | 12.148 | / | / | 0.42 | 0.103 | / | / | / | / | / | / | / | 1.009 | remainder | 0.1764 | 0.0492 | 0.0404 |
| Embodim ent 48 | / | / | 17.352 | 14.151 | / | / | 0.441 | 0.202 | / | / | / | / | / | / | / | 1.011 | remainder | 0.1843 | 0.0501 | 0.0378 |
| Embodim ent 49 | / | / | 15.352 | 16.152 | / | / | 0.501 | 0.302 | / | / | / | / | / | / | / | 1.010 | remainder | 0.1973 | 0.0529 | 0.0347 |
| Embodim ent 50 | / | / | 14.352 | 17.152 | / | / | 0.34 | 0.403 | / | / | / | / | / | / | / | 1.010 | remainder | 0.2147 | 0.0564 | 0.307 |
| Embodim ent 51 | / | / | 12.352 | 19.148 | / | / | 0.381 | 0.501 | / | / | / | / | / | / | / | 1.009 | remainder | 0.2251 | 0.0588 | 0.029 |
| Embodim ent 52 | / | / | 11.351 | 20.148 | / | / | 0.42 | 0.602 | / | / | / | / | / | / | / | 1.011 | remainder | 0.2248 | 0.0641 | 0.0256 |
| Embodim ent 53 | / | / | 9.352 | 22.149 | / | / | 0.341 | 0.502 | 0.102 | / | / | / | / | / | / | 1.010 | remainder | 0.2379 | 0.0675 | 0.0228 |
| Embodim ent 54 | / | / | 7.353 | 24.148 | / | / | 0.401 | 0.602 | 0.302 | / | / | / | / | / | / | 1.009 | remainder | 0.2456 | 0.0691 | 0.0187 |
| Embodim ent 55 | / | / | 13.653 | 17.152 | / | / | 0.501 | 0.81 | 0.421 | / | / | / | / | / | / | 1.010 | remainder | 0.1761 | 0.0494 | 0.0398 |
| Embodim ent 56 | / | / | 8.651 | 22.151 | / | / | 0.341 | 0.501 | 0.102 | / | 0.25 | / | / | / | / | 1.009 | remainder | 0.184 | 0.0503 | 0.0371 |
| Embodim ent 57 | / | / | 6.652 | 24.151 | / | / | 0.501 | 0.802 | 0.302 | / | 0.30 | / | / | / | / | 1.011 | remainder | 0.1761 | 0.0494 | 0.0397 |
| Embodim ent 58 | / | / | 21.951 | 8.846 | / | / | 0.34 | 0.01 | 0.251 | / | / | / | / | / | / | 1.010 | remainder | 0.1846 | 0.05 | 0.0366 |
| Embodim ent 59 | / | / | 20.652 | 10.148 | / | / | 0.381 | 0.021 | 0.302 | / | / | / | / | / | / | 0.962 | remainder | 0.1069 | 0.0384 | 0.0476 |
| Embodim ent 60 | / | / | 18.652 | 12.15 | / | / | 0.421 | 0.03 | 0.42 | / | / | / | / | / | / | 0.958 | remainder | 0.1253 | 0.0444 | 0.0455 |
| Embodim ent 61 | / | / | 16.651 | 14.147 | / | / | 0.382 | 0.042 | 0.102 | / | / | / | / | / | / | 0.958 | remainder | 0.1534 | 0.0458 | 0.0436 |
| Embodim ent 62 | / | / | 14.652 | 16.148 | / | / | 0.420 2 | 0.102 | 0.151 | / | / | / | / | / | / | 0.958 | remainder | 0.1761 | 0.0494 | 0.0398 |
| Embodim ent 63 | / | / | 13.651 | 17.149 | / | / | 0.441 | 0.202 | 0.251 | / | / | / | / | / | / | 0.958 | remainder | 0.184 | 0.0503 | 0.0372 |
| Embodim ent 64 | / | / | 11.652 | 19.152 | / | / | 0.502 | 0.302 | 0.301 | / | / | / | / | / | / | 0.961 | remainder | 0.197 | 0.0531 | 0.0341 |
| Embodim ent 65 | / | / | 10.651 | 20.149 | / | / | 0.451 | 0.402 | 0.421 | / | / | / | / | / | / | 0.985 | remainder | 0.2144 | 0.0566 | 0.0301 |
| Embodim ent 66 | / | / | 8.652 | 22.149 | / | / | 0.502 | 0.502 | 0.502 | / | / | / | / | / | / | 1.009 | remainder | 0.2248 | 0.059 | 0.0284 |
| Embodim ent 67 | / | / | 12.651 | 18.151 | / | / | 0.401 | 0.602 | 0.401 | 2.501 | 0.302 | / | / | Cr | 0.05 | 1.011 | remainder | 0.2245 | 0.0643 | 0.025 |
| Embodim ent 68 | / | / | 12.652 | 18.152 | / | / | 0.403 | 0.601 | 0.401 | 2.501 | 0.302 | / | / | Cr | 0.12 | 1.012 | remainder | 0.1062 | 0.039 | 0.0482 |
| Embodim ent 69 | / | / | 13.649 | 17.151 | Dy | 1.51 | 0.403 | 0.302 | 0.301 | 2.502 | 0.301 | / | / | / | / | 1.011 | remainder | 0.1251 | 0.0412 | 0.0458 |
| Embodim ent 70 | / | / | 12.649 | 18.152 | Dy | 2.011 | 0.4 | 0.298 | 0.301 | 2.502 | 0.302 | / | / | / | / | 0.958 | remainder | 0.1532 | 0.0432 | 0.0439 |
| Embodim ent 71 | / | / | 11.651 | 19.152 | Dy | 2.511 | 0.41 | 0.351 | 0.30 | 2.501 | 0.303 | / | / | / | / | 0.961 | remainder | 0.1759 | 0.0468 | 0.0401 |
| Embodim ent 72 | / | / | 11.652 | 19.151 | Dy | 2.512 | 0.402 | 0.451 | 0.302 | 2.501 | 0.303 | / | / | / | / | 0.962 | remainder | 0.1835 | 0.0493 | 0.0375 |
| Embodim ent 73 | / | / | 13.651 | 17.152 | Tb | 1.991 | 0.402 | 0.302 | 0.301 | 2.505 | 0.303 | / | / | / | / | 0.958 | remainder | 0.1965 | 0.0523 | 0.0342 |
| Embodim ent 74 | / | / | 12.650 | 18.151 | Tb | 1.212 | 0.402 | 0.302 | 0.301 | 2.501 | 0.308 | / | / | / | / | 0.961 | remainder | 0.2139 | 0.0558 | 0.0302 |
| Embodim ent 75 | Ce | 0.29 | 11.352 | 18.152 | Tb | 1.219 | 0.41 | 0.601 | 0.399 | 2.491 | 0.298 | / | / | / | / | 0.962 | remainder | 0.2234 | 0.0582 | 0.0085 |
| Embodim ent 76 | / | / | 21.647 | 8.848 | Dy | 0.62 | / | / | / | / | / | / | / | / | / | 0.947 | remainder | 0.1075 | 0.041 | 0.0485 |
| Embodim ent 77 | / | / | 21.649 | 8.846 | Tb | 0.58 | / | / | / | / | / | / | / | / | / | 0.946 | remainder | 0.1069 | 0.0391 | 0.0486 |
| Comparat ive Embodim ent 1 | / | / | 21.998 | 7.988 | / | / | / | / | / | / | / | / | / | / | / | 0.958 | remainder | 0.2248 | 0.0635 | 0.0251 |
| Comparat ive Embodim ent 2 | / | / | 22.094 | 7.989 | / | / | 0.401 | 0 | 0.403 | 2.489 | 0.289 | / | / | Cr | 0.121 | 0.961 | remainder | 0.2379 | 0.0669 | 0.0223 |

(3) Fe-EPMA detection: The vertical orientation surfaces of the RTB-based magnet materials in Embodiments 1, 2, 11, 12, 21, 23, 34, 35, 39, 43, 51, 52, 60, 63, 68, 69 and Comparative Embodiments 1 and 2 in Table 4 were polished. Field emission electron probe microanalyzer (FE-EPMA) (JEOL, 8530F) was used for detection.

The position of intergranular triangle region in Embodiment 68 (as shown at position a in Figure 1) was investigated for composition, and the relative volume ratio of the phase of the triangle region (rare-earth-rich phase) to all phases of the observation surface (main phase, the grain boundary phase and the rare-earth-rich phase) was determined, which can be found that in the samples containing high Pr and high C, the ration of the phases formed in intergranular region was relatively low, which was not seen in the samples containing low Pr. The specific test results are shown in Table 5 below.

**Table 5**

| No. | Intergranular triangle region | | | Proportion of phases in the Intergranular triangle region |
|---|---|---|---|---|
| | R' (mass ratio) | Ga+Cu (mass ratio) | O (mass ratio) | / |
| Embodiment 1 | 85.4 | / | 14.6 | 4.6 |
| Embodiment 2 | 85.3 | / | 14.7 | 5.3 |
| Embodiment 11 | 85.3 | / | 14.7 | 4.8 |
| Embodiment 12 | 85.4 | 0.9 (Cu) | 13.7 | 3.2 |
| Embodiment 21 | 85.3 | / | 14.7 | 3.3 |
| Embodiment 23 | 85.3 | / | 14.7 | 4.6 |
| Embodiment 34 | 85.2 | 0.4 (Ga) | 14.4 | 4.8 |
| Embodiment 35 | 85 | 0.6 (Ga) | 14.4 | 3.7 |
| Embodiment 39 | 85.2 | / | 14.8 | 3.2 |
| Embodiment 43 | 85.3 | / | 14.7 | 3.3 |
| Embodiment 51 | 84.9 | 0.8 (Cu) | 14.3 | 4.6 |
| Embodiment 52 | 84.9 | 0.6 (Cu) | 14.5 | 4.8 |
| Embodiment 60 | 84.35 | 0.3 (Cu)+ 0.6 (Ga) | 14.75 | 3.2 |
| Embodiment 63 | 84.8 | 0.4 (Cu)+ 0.4 (Ga) | 14.4 | 3.3 |
| Embodiment 68 | 85.85 | 0.4 (Cu)+ 0.5 (Ga) | 13.25 | 4.6 |
| Embodiment 69 | 84.8 | 0.4 (Cu)+ 0.6 (Ga) | 14.2 | 4.8 |
| Comparative Embodiment 1 | 85.3 | / | 14.7 | 9.8 |
| Comparative Embodiment 2 | 84.7 | 0.4 (Cu)+ 0.6 (Ga) | 14.3 | 12.5 |

| | | | | |
|---|---|---|---|---|
| Note: The mass ratio of R', Ga, Cu and O in the intergranular triangle region refers to the mass percentage in the total mass of elements in the intergranular triangle region; the volume ratio of the phase in intergranular triangle region refers to the percentage of the volume of the phase in intergranular triangle region with respect to the sum of the volume of the "main phase, the grain boundary phase and the intergranular triangle region". | | | | |

## Claims

1. A preparation method for an RTB-based permanent magnet material, wherein the preparation method comprises the following steps: the molten liquid of the raw material composition of the RTB-based permanent magnet material is subjected to casting, hydrogen decrepitation, and pulverization to obtain a powder, and the powder is mixed with dispersant, and then pressed, formed, sintered and aged; wherein:
(1) the raw material composition of RTB-based permanent magnet material comprises the following components by mass percentage:
R': 29.5-33.5 wt.%, R' is a rare earth element, R' comprises Pr, the content of Pr is >_8.85 wt.%;
X: 0-5.0 wt.%, X is one or more of Cu, Al, Ga, Co, Zr, Ti, Nb and Mn;
B: 0.90-1.2 wt.%;
Fe: 61.4-69.5 wt.%;
(2) in the process of pulverization, O ≤ 60 ppm in the pulverization atmosphere;
(3) in the pressing process, O ≤ 40 ppm in the pressing atmosphere;
(4) the dispersant comprises element C, and the mass percentage of the dispersant in the mixed powder is 0.04-0.2%;
the molten liquid of the raw material composition of the RTB-based permanent magnet material is prepared by the following method: melting in a vacuum induction melting furnace; the vacuum degree of the melting furnace is 5×10⁻² Pa; the melting temperature is below 1500°C;
the casting process is carried out as follows: cooling at a rate of 10²°C /s -10⁴°C/s in an Ar atmosphere;
the pulverization is jet mill pulverization; the pressure in the pulverization chamber of the jet mill pulverization is 0.38 MPa; the time of the jet mill pulverization is 3 hours;
the sintering is also preceded by preheating; wherein, the temperature of the preheating is 300-600°C, the time of the preheating is 1-2h; preferably, the preheating is preheating at 300°C and 600°C for 1h respectively;
the temperature of the sintering is 1040-1090°C;
the time of the sintering is 2h;
the grain boundary diffusion treatment is also carried out after sintering and before the aging treatment; wherein, preferably, the grain boundary diffusion treatment is carried out according to the following steps, attaching substance containing Tb and/or containing Dy to the surface of the RTB-based permanent magnet material by evaporating, coating or sputtering, then carrying out diffusion heat treatment; the temperature of the diffusion heat treatment is preferably 800-900°C; the time of the diffusion heat treatment is preferably 12-48h;
the treatment temperature of the aging treatment is 500-650°C;
in the aging treatment, the heating rate of heating to 500-650°C is 3-5 °C/min;
the treatment time of the aging treatment is 3h.

2. The preparation method of RTB-based permanent magnet material according to claim 1, wherein, the content of R' is 29.5-33.3 wt.%, preferably 9.5 wt.%, 30.5 wt.%, 30.8 wt.%, 31 wt.%, 31.5 wt.%, 32 wt.%, 32.3 wt.%, 32.8 wt.% or 33.3 wt.%, the percentage refers to the mass percentage in the raw material composition of the RTB-based permanent magnet material;
the content of Pr is 8.85-27.15 wt.%, such as 8.85 wt.%, 9.85 wt.%, 10.15 wt.%, 10.85 wt.%, 11.85 wt.%, 12.15 wt.%, 13.15 wt.%, 14.15 wt.%, 16.15 wt.%, 17.15 wt.%, 18.15 wt.%, 19.15 wt.%, 20.15 wt.%, 21.15 wt.%, 22.15 wt.%, 23.15 wt.%, 24.15 wt.%, 25.15 wt.% or 27.15 wt.%, the percentage refers to the mass percentage in the raw material composition of the RTB-based permanent magnet material;
R' further comprises Nd and/or R, R is a rare earth element besides Pr and Nd; wherein, the content of NO is preferably 3.35-22.65 wt.%, more preferably 3.35 wt.%, 5.35 wt.%, 6.65 wt.%, 6.85 wt.%, 7.35 wt.%, 7.85 wt.%, 8.35 wt.%, 8.65 wt.%, 8.85 wt.%, 9.35 wt.%, 10.65 wt.%, 10.85 wt.%, 11.35 wt.%, 11.65 wt.%, 11.85 wt.%, 12.35 wt.%, 12.65 wt.%, 13.35 wt.%, 13.65 wt.%, 13.85 wt.%, 14.35 wt.%, 14.65 wt.%, 14.8 wt.5%, 15.35 wt.%, 16.35 wt.%, 16.65 wt.%, 16.85 wt.%, 17.35 wt.%, 17.65 wt.%, 18.35 wt.%, 18.65 wt.%, 18.85 wt.%, 19.35 wt.%, 19.65 wt.%, 20.65 wt.%, 20.85 wt.%, 21.35 wt.%, 21.65 wt.%, 21.95 wt.%, 22.15 wt.% or 22.65 wt.%, the percentage refers to the mass percentage in the raw material composition of the RTB-based permanent magnet material; the mass ratio of Nd to R' is preferably ≤0.72; the kind of R is preferably Y and/or Ce; the content of R is preferably 0-1 wt.%, for example 0.3 wt.%, the percentage refers to the mass percentage in the raw material composition of the RTB-based permanent magnet material;
R' further comprises a heavy rare earth element RH; the kind of RH is preferably Dy and/or Tb; the content of RH is preferably 1.2-2.5 wt.%, such as 1.2 wt.%, 1.5 wt.%, 2 wt.% or 2.5 wt.%, and the percentage refers to the mass percentage in the raw material composition of the RTB-based permanent magnet material; the mass ratio of RH to R' is preferably < 0.253, for example 0.038-0.075, and then 0.038, 0.039, 0.046, 0.061 or 0.075; when the RH comprises Tb, the content of Tb is preferably 1.2-2.0 wt.%, for example 1.2 wt.% or 2.0 wt.%, the percentage refers to the mass percentage in the raw material composition of the RTB-based permanent magnet material; when the RH comprises Dy, the content of Dy is preferably 1.5-2.5 wt.%, such as 1.5 wt.%, 2.0 wt.% or 2.5 wt.%, the percentage refers to the mass percentage in the raw material composition of the RTB-based permanent magnet material;
the content of B is 0.95-1.1 wt.%, such as 0.95 wt.%, 0.96 wt.%, 0.98 wt.% or 1.01 wt.%, the percentage refers to the mass percentage in the raw material composition of the RTB-based permanent magnet material;
the content of Fe is 61.5-69.5 wt.%, such as 61.79 wt.%, 61.89 wt.%, 62.44 wt.%, 62.89 wt.%, 63.24 wt.%, 63.84 wt.%, 63.87 wt.%, 63.94 wt.%, 64.99 wt.%, 66.19 wt.%, 66.29 wt.%, 66.47 wt.%, 66.52 wt.%, 66.55 wt.%, 66.61 wt.%, 66.69 wt.%, 66.75 wt.%, 66.85 wt.%, 66.97 wt.%, 67.00 wt.%, 67.02 wt.%, 67.068 wt.%, 67.13 wt.%, 67.14 wt.%, 67.19 wt.%, 67.24 wt.%, 67.25 wt.%, 67.35 wt.%, 67.37 wt.%, 67.45 wt.%, 67.49 wt.%, 67.54 wt.%, 67.55 wt.%, 67.57 wt.%, 67.59 wt.%, 67.64 wt.%, 67.65 wt.%, 67.69 wt.%, 67.718 wt.%, 67.75 wt.%, 67.85 wt.%, 67.95 wt.%, 67.96 wt.%, 67.97 wt.%, 68.008 wt.%, 68.12 wt.%, 68.55 wt.%, 68.62 wt.%, 69.02 wt.%, 69.1 wt.%, 69.22 wt.%, 69.27 wt.%, 69.32 wt.% or 69.45 wt.%, the percentage refers to the mass percentage in the raw material composition of the RTB-based permanent magnet material; X is Cu, Al, Ga, Co, Zr, Ti or Nb, or, "Cu and Al", "Ga and Mn", "Cu, Al and Ga", "Cu, Al, Ga and Zr", "Cu, Al, Ga and Co" or "Cu, Al, Ga, Zr and Co";
the content of the X is 0-4.5 wt.%; when X comprises Cu, the content of the Cu is preferably 0.2-0.5 wt.%; when the X comprises Al, the content of Al is preferably 0-0.8 wt.%, but not 0, such as 0.01-0.03 wt.% or 0.5-0.8 wt.%; when the X comprises Ga, the content of Ga is preferably 0.0-1.85 wt.%, but not 0, and more preferably 0.1-1.55 wt.%; when the X comprises Co, the content of Co is preferably 0.0-3.0 wt.%, but not 0, and more preferably 0.5-2.5 wt.%; when the X comprises Zr, the content of Zr is preferably 0.25-0.35 wt.%; when the X comprises Nb, the content of Nb is preferably 0.25-0.35 wt.%; when the X comprises Mn, the content of Mn is preferably 0.0-0.03 wt.%, but not 0; the percentage refers to the mass percentage in the raw material composition of the RTB-based permanent magnet material;
the RTB-based permanent magnet material further comprises M, M is one or more of Ni, Zn, Ag, In, Sn, Bi, V, Cr, Hf, Ta and W; wherein, the kind of M is preferably Cr; the content of M is preferably 0-0.15 wt.%, but not 0, and the percentage refers to the mass percentage in the raw material composition of the RTB-based permanent magnet material.

3. The preparation method of RTB-based permanent magnet material according to claim 1 or 2, wherein, during the process of pulverization, the content of oxygen O in the pulverization atmosphere is 0-50 ppm, such as 0 ppm, 5 ppm, 10 ppm, 15 ppm, 20 ppm, 25 ppm, 30 ppm, 35 ppm, 40 ppm, 45 ppm, or 50 ppm;
the dispersant is a lubricant and/or an antioxidant, preferably the lubricant is zinc stearate; when the dispersant contains zinc stearate, the amount of zinc stearate can be 0.04-0.14%, such as 0.04%, 0.05%, 0.06%, 0.07%, 0.08%, 0.09%, 0.1%, 0.11%, 0.12%, 0.13% or 0.14%, the percentage refers to the mass percentage with respect to the total mass of the mixed powder; the content of the dispersant is 0.04-0.14%, such as 0.04%, 0.05%, 0.06%, 0.07%, 0.08%, 0.09%, 0.1%, 0.11%, 0.12%, 0.13% or 0.14%, the percentage refers to the mass percentage with respect to the total mass of the mixed powder;
during the pressing process, the content of oxygen O in the pressing atmosphere is 10-30 ppm, such as 10 ppm, 12 ppm, 14 ppm, 16 ppm, 18 ppm, 20 ppm, 22 ppm, 24 ppm, 26 ppm, 28 ppm, or 30 ppm.

## Patentansprüche

1. Ein Herstellungsverfahren für ein Dauermagnetmaterial auf RTB-Basis, wobei das Herstellungsverfahren die folgenden Schritte umfasst: Die geschmolzene Flüssigkeit der Rohmaterialzusammensetzung des Dauermagnetmaterials auf RTB-Basis wird einem Gießvorgang, einer Wasserstoffdekrepitation und einer Pulverisierung unterzogen, um ein Pulver zu erhalten, und das Pulver wird mit einem Dispergiermittel gemischt und dann gepresst, geformt, gesintert und gealtert; wobei:
(1) die Rohmaterialzusammensetzung des Dauermagnetmaterials auf RTB-Basis umfasst die folgenden Komponenten in Massenprozent:
R': 29,5-33,5 Gew.-%, R' ist ein Seltenerdelement, R' umfasst Pr, der Gehalt an Pr beträgt ≥8,85 Gew.-%;
X: 0-5,0 Gew.-%, X ist eines oder mehrere von Cu, Al, Ga, Co, Zr, Ti, Nb und Mn;
B: 0,90-1,2 Gew.-%;
Fe: 61,4-69,5 Gew.-%;
(2) beim Pulverisierungsvorgang ist O ≤ 60 ppm in der Pulverisierungsatmosphäre;
(3) beim Pressvorgang ist O ≤ 40 ppm in der Pressatmosphäre;
(4) das Dispergiermittel umfasst das Element C und der Massenprozentsatz des Dispergiermittels in dem gemischten Pulver beträgt 0,04-0,2%;
die geschmolzene Flüssigkeit der Rohmaterialzusammensetzung des Dauermagnetmaterials auf RTB-Basis wird nach folgendem Verfahren hergestellt: Schmelzen in einem Vakuum-Induktionsschmelzofen; der Vakuumgrad des Schmelzofens beträgt 5×10⁻² Pa; die Schmelztemperatur liegt unter 1500°C;
der Gießvorgang wird wie folgt durchgeführt: Abkühlung mit einer Rate von 10² °C /s -10⁴ °C/s in einer Ar-Atmosphäre;
die Pulverisierung ist eine Strahlmühl-Pulverisierung; der Druck in der Pulverisierungskammer der Strahlmühle beträgt 0,38 MPa; die Dauer des Strahlmühl-Pulverisierens beträgt 3 Stunden;
dem Sintern geht auch ein Vorheizen voraus, wobei die Temperatur des Vorheizens 300-600°C und die Dauer des Vorheizens 1-2h beträgt; vorzugsweise ist das Vorheizen ein Vorheizen bei 300°C und 600°C für jeweils 1h;
die Sintertemperatur beträgt 1040-1090°C;
die Dauer der Sinterung beträgt 2 Stunden;
die Korngrenzen-Diffusionsbehandlung wird ebenfalls nach dem Sintern und vor der Alterungsbehandlung durchgeführt; wobei die Korngrenzen-Diffusionsbehandlung vorzugsweise gemäß den folgenden Schritten durchgeführt wird: Aufbringen einer Tb-und/oder Dy-haltigen Substanz auf die Oberfläche des Dauermagnetmaterials auf RTB-Basis durch Aufdampfen, Beschichten oder Sputtern, dann Durchführung einer Diffusionswärmebehandlung; die Temperatur der Diffusionswärmebehandlung beträgt vorzugsweise 800-900°C; die Dauer der Diffusionswärmebehandlung beträgt vorzugsweise 12-48h;
die Behandlungstemperatur bei der Alterungsbehandlung beträgt 500-650°C;
bei der Alterungsbehandlung beträgt die Erhitzungsrate auf 500-650 °C 3-5 °C/min;
die Behandlungsdauer bei der Alterungsbehandlung beträgt 3 Stunden.

2. Herstellungsverfahren für ein Dauermagnetmaterial auf RTB-Basis nach Anspruch 1, wobei der Gehalt an R' 29,5-33,3 Gew.-%, vorzugsweise 9,5 Gew.-%, 30,5 Gew.-%, 30,8 Gew.-%, 31 Gew.-%, 31,5 Gew.-%, 32 Gew.-%, 32,3 Gew.-%, 32,8 Gew.-% oder 33,3 Gew.-% beträgt, wobei sich der Prozentsatz auf den Massenprozentsatz in der Rohmaterialzusammensetzung des Dauermagnetmaterials auf RTB-Basis bezieht;
der Gehalt an Pr beträgt 8,85-27,15 Gew.-%, wie 8,85 Gew.-%, 9,85 Gew.-%, 10,15 Gew.-%, 10,85 Gew.-%, 11,85 Gew.-%, 12,15 Gew.-%, 13,15 Gew.-%, 14,15 Gew.-%, 16,15 Gew.-%, 17,15 Gew.-%, 18,15 Gew.-%, 19,15 Gew.-%, 20,15 Gew.-%, 21,15 Gew.-%, 22,15 Gew.-%, 23,15 Gew.-%, 24,15 Gew.-%, 25,15 Gew.-% oder 27,15 Gew.-%.%, 21,15 Gew.-%, 22,15 Gew.-%, 23,15 Gew.-%, 24,15 Gew.-%, 25,15 Gew.-% oder 27,15 Gew.-%, wobei sich der Prozentsatz auf den Massenprozentsatz in der Rohmaterialzusammensetzung des Dauermagnetmaterials auf RTB-Basis bezieht;
R' umfasst ferner Nd and/or R, R ist ein Seltenerdelement außer Pr and Nd; wobei der Gehalt an Nd vorzugsweise 3,35-22,65 Gew.-%, mehr bevorzugt 3,35 Gew.-%, 5,35 Gew.-%, 6,65 Gew.-%, 6,85 Gew.-%, 7,35 Gew.-%, 7,85 Gew.-%, 8,35 Gew.-%, 8,65 Gew.-%, 8,85 Gew.-%, 9,35 Gew.-%, 10,65 Gew.-%, 10,85 Gew.-%, 11,35 Gew.-%, 11,65 Gew.-%, 11,85 Gew.-%, 12,35 Gew.-%, 12,65 Gew.-%, 13,35 Gew.-%, 13,65 Gew.-%, 13,85 Gew.-%, 14,35 Gew.-%, 14,65 Gew.-%, 14,85 Gew.-%, 15,35 Gew.-%, 16,35 Gew.-%, 16,65 Gew.-%, 16,85 Gew.-%, 17,35 Gew.-%, 17,65 Gew.-%, 18,35 Gew.-%, 18,65 Gew.-%, 18,85 Gew.-%, 19,35 Gew.-%, 19,65 Gew.-%, 20,65 Gew.-%, 20,85 Gew.-%, 21,35 Gew.-%, 21,65 Gew.-%, 21,95 Gew.-%, 22,15 Gew.-% oder 22,65 Gew.-% beträgt, wobei sich der Prozentsatz auf den Massenprozentsatz in der Rohmaterialzusammensetzung des Dauermagnetmaterials auf RTB-Basis bezieht; das Massenverhältnis von Nd zu R' ist vorzugsweise ≤0,72; die Art von R ist vorzugsweise Y und/oder Ce; der Gehalt an R beträgt vorzugsweise 0-1 Gew.-%, zum Beispiel 0,3 Gew.-%, wobei sich der Prozentsatz auf den Massenprozentsatz in der Rohmaterialzusammensetzung des Dauermagnetmaterials auf RTB-Basis bezieht;
R' umfasst ferner ein schweres Seltenerdelement RH; die Art von RH ist vorzugsweise Dy und/oder Tb; der Gehalt an RH beträgt vorzugsweise 1,2-2,5 Gew.-%, wie 1,2 Gew.-%, 1,5 Gew.-%, 2 Gew.-% oder 2,5 Gew.-%, und der Prozentsatz bezieht sich auf den Massenprozentsatz in der Rohmaterialzusammensetzung des Dauermagnetmaterials auf RTB-Basis; das Massenverhältnis von RH zu R' ist vorzugsweise < 0,253, zum Beispiel 0,038-0,075, und dann 0,038, 0,039, 0,046, 0,061 oder 0,075; wenn RH Tb umfasst, ist der Gehalt an Tb vorzugsweise 1,2-2,0 Gew.-%, zum Beispiel 1,2 Gew.-% oder 2,0 Gew.-%, wobei sich der Prozentsatz auf den Massenprozentsatz in der Rohmaterialzusammensetzung des Dauermagnetmaterials auf RTB-Basis bezieht; wenn RH Dy umfasst, ist der Gehalt an Dy vorzugsweise 1,5-2,5 Gew.-%, wie 1,5 Gew.-%, 2,0 Gew.-% oder 2,5 Gew.-%, wobei sich der Prozentsatz auf den Massenprozentsatz in der Rohmaterialzusammensetzung des Dauermagnetmaterials auf RTB-Basis bezieht;
der Gehalt an B beträgt 0,95-1,1 Gew.-%, wie 0,95 Gew.-%, 0,96 Gew.-%, 0,98 Gew.-% oder 1,01 Gew.-%, wobei sich der Prozentsatz auf den Massenprozentsatz in der Rohmaterialzusammensetzung des Dauermagnetmaterials auf RTB-Basis bezieht;
der Fe-Gehalt beträgt 61,5-69,5 Gew.-%, wie 61,79 Gew.-%, 61,89 Gew.-%, 62,44 Gew.-%, 62,89 Gew.-%, 63,24 Gew.-%, 63,84 Gew.-%, 63,87 Gew.-%, 63,94 Gew.-%, 64,99 Gew.-%, 66,19 Gew.-%, 66,29 Gew.-%, 66,47 Gew.-%, 66,52 Gew.-%, 66,55 Gew.-%, 66,61 Gew.-%, 66,69 Gew.-%, 66,75 Gew.-%, 66,85 Gew.-%, 66,97 Gew.-%, 67,00 Gew.-%, 67,02 Gew.-%, 67,068 Gew.-%, 67,13 Gew.-%, 67,14 Gew.-%, 67,19 Gew.-%, 67,24 Gew.-%, 67,25 Gew.-%, 67,35 Gew.-%, 67,37 Gew.-%, 67,45 Gew.-%, 67,49 Gew.-%, 67,54 Gew.-%, 67,55 Gew.-%, 67,57 Gew.-%, 67,59 Gew.-%, 67,64 Gew.-%, 67,65 Gew.-%, 67,69 Gew.-%, 67,718 Gew.-%, 67,75 Gew.-%, 67,85 Gew.-%, 67,95 Gew.-%, 67,96 Gew.-%, 67,97 Gew.-%, 68,008 Gew.-%, 68,12 Gew.-%, 68,55 Gew.-%, 68,62 Gew.-%, 69,02 Gew.-%, 69,1 Gew.-%, 69,22 Gew.-%, 69,27 Gew.-%, 69,32 Gew.-% oder 69,45 Gew.-%, wobei sich der Prozentsatz auf den Massenprozentsatz in der Rohmaterialzusammensetzung des Dauermagnetmaterials auf RTB-Basis bezieht;
X ist Cu, Al, Ga, Co, Zr, Ti oder Nb, oder "Cu und Al", "Ga und Mn", "Cu, Al und Ga", "Cu, Al, Ga und Zr", "Cu, Al, Ga und Co" oder "Cu, Al, Ga, Zr und Co";
der Gehalt an X beträgt 0-4,5 Gew.-%; wenn X Cu umfasst, beträgt der Gehalt an Cu vorzugsweise 0,2-0,5 Gew.-%; wenn X Al umfasst, beträgt der Gehalt an Al vorzugsweise 0-0,8 Gew.-%, jedoch nicht 0, wie zum Beispiel 0,01-0,03 Gew.-% oder 0,5-0,8 Gew.-%; wenn X Ga umfasst, beträgt der Gehalt an Ga vorzugsweise 0,0-1,85 Gew.-%, aber nicht 0, und mehr bevorzugt 0,1-1,55 Gew.-%; wenn X Co umfasst, beträgt der Gehalt an Co vorzugsweise 0,0-3,0 Gew.-%, aber nicht 0, und mehr bevorzugt 0,5-2,5 Gew.-%; wenn X Zr umfasst, beträgt der Gehalt an Zr vorzugsweise 0,25-0,35 Gew.-%; wenn X Nb umfasst, beträgt der Gehalt an Nb vorzugsweise 0,25-0,35 Gew.-%; wenn X Mn umfasst, beträgt der Gehalt an Mn vorzugsweise 0,0-0,03 Gew.-%, aber nicht 0; der Prozentsatz bezieht sich auf den Massenprozentsatz in der Rohmaterialzusammensetzung des Dauermagnetmaterials auf RTB-Basis;
das Dauermagnetmaterial auf RTB-Basis umfasst ferner M, M ist eines oder mehrere von Ni, Zn, Ag, In, Sn, Bi, V, Cr, Hf, Ta und W; wobei die Art von M vorzugsweise Cr ist, der Gehalt an M vorzugsweise 0-0,15 Gew.-%, aber nicht 0 ist, und der Prozentsatz sich auf den Massenprozentsatz in der Rohmaterialzusammensetzung des Dauermagnetmaterials auf RTB-Basis bezieht.

3. Herstellungsverfahren für ein Dauermagnetmaterial auf RTB-Basis nach Anspruch 1 oder 2, wobei während des Pulverisierungsvorgangs der Gehalt an Sauerstoff O in der Pulverisierungsatmosphäre 0-50 ppm beträgt, wie zum Beispiel 0 ppm, 5 ppm, 10 ppm, 15 ppm, 20 ppm, 25 ppm, 30 ppm, 35 ppm, 40 ppm, 45 ppm oder 50 ppm;
das Dispergiermittel ist ein Schmiermittel und/oder ein Antioxidationsmittel, vorzugsweise ist das Schmiermittel Zinkstearat; wenn das Dispergiermittel Zinkstearat enthält, kann die Menge an Zinkstearat 0,04-0,14% betragen, wie zum Beispiel 0,04%, 0,05%, 0,06%, 0,07%, 0,08%, 0,09%, 0,1%, 0,11%, 0,12%, 0,13% oder 0,14%, wobei sich der Prozentsatz auf den Massenprozentsatz bezogen auf die Gesamtmasse des gemischten Pulvers bezieht;
der Gehalt an Dispergiermittel beträgt 0,04-0,14%, wie zum Beispiel 0,04%, 0,05%, 0,06%, 0,07%, 0,08%, 0,09%, 0,1%, 0,11%, 0,12%, 0,13% oder 0,14%, wobei sich der Prozentsatz auf den Massenprozentsatz bezogen auf die Gesamtmasse des gemischten Pulvers bezieht; während des Pressvorgangs beträgt der Gehalt an Sauerstoff O in der Pressatmosphäre 10-30 ppm, zum Beispiel 10 ppm, 12 ppm, 14 ppm, 16 ppm, 18 ppm, 20 ppm, 22 ppm, 24 ppm, 26 ppm, 28 ppm oder 30 ppm.

## Revendications

1. Procédé de préparation pour un matériau d'aimant permanent à base de RTB, le procédé de préparation comprenant les étapes suivantes : le liquide fondu de la composition de matière première du matériau d'aimant permanent à base de RTB étant soumis à une coulée, une décrépitation à l'hydrogène et une pulvérisation pour obtenir une poudre, et la poudre étant mélangée avec un dispersant et ensuite pressée, formée, frittée et vieillie ;
(1) la composition de matière première du matériau d'aimant permanent à base de RTB comprenant les composants suivants par pourcentage en masse :
R' : 29,5-33,5 % en poids, R' étant un élément des terres rares, R' comprenant du Pr, la teneur en Pr étant ≥ 8,85 % en poids ;
X : 0-5,0 % en poids, X étant un ou plusieurs éléments parmi Cu, Al, Ga, Co, Zr, Ti, Nb et Mn ;
B : 0,90-1,2 % en poids ;
Fe : 61,4-69,5 % en poids ;
(2) dans le processus de pulvérisation, O ≤ 60 ppm dans l'atmosphère de pulvérisation ;
(3) dans le processus de pressage, O ≤ 40 ppm dans l'atmosphère de pressage ;
(4) le dispersant comprenant l'élément C, et le pourcentage en masse du dispersant dans la poudre mélangée étant de 0,04 à 0,2 % ;
le liquide fondu de la composition de matière première du matériau d'aimant permanent à base de RTB étant préparé par le procédé suivant : fusion dans un fourneau de fusion par induction sous vide ; le degré de vide du fourneau de fusion étant de 5 × 10⁻² Pa ; la température de fusion étant inférieure à 1 500 °C ;
le processus de coulée étant réalisé comme suit : refroidissement à une vitesse de 10² °C/s à 10⁴ °C/s dans une atmosphère d'Ar ;
la pulvérisation étant une pulvérisation par un broyeur à jet ; la pression dans le compartiment de pulvérisation de la pulvérisation par un broyeur à jet étant de 0,38 MPa ; la durée de la pulvérisation par un broyeur à jet étant de 3 heures ;
le frittage étant également précédé par un préchauffage ; la température du préchauffage étant de 300 à 600 °C, la durée du préchauffage étant de 1 à 2 h ; préférablement, le préchauffage étant un préchauffage à 300 °C et 600 °C pendant 1 h respectivement ;
la température du frittage étant de 1 040 à 1 090 °C ;
la durée du frittage étant de 2 h ;
le traitement par diffusion intragranulaire étant également réalisé après frittage et avant le traitement de vieillissement ; préférablement le traitement par diffusion intragranulaire étant réalisé selon les étapes suivantes : fixation d'une substance contenant du Tb et/ou contenant du Dy sur la surface du matériau d'aimant permanent à base de RTB par évaporation, revêtement ou pulvérisation, puis réalisation d'un traitement thermique par diffusion ; la température du traitement thermique par diffusion étant préférablement de 800 à 900 °C ; la durée du traitement thermique par diffusion étant préférablement de 12 à 48 h ;
la température de traitement du traitement de vieillissement étant de 500 à 650 °C ;
dans le traitement de vieillissement, la vitesse de chauffage du chauffage jusqu'à une température de 500 à 650 °C étant de 3 à 5 °C/min ;
la durée de traitement du traitement de vieillissement étant de 3 h.

2. Procédé de préparation pour un matériau d'aimant permanent à base de RTB selon la revendication 1, la teneur en R' étant de 29,5-33,3 % en poids, préférablement de 9,5 % en poids, 30,5 % en poids, 30,8 % en poids, 31 % en poids, 31,5 % en poids, 32 % en poids, 32,3 % en poids, 32,8 % en poids ou 33,3 % en poids, le pourcentage faisant référence au pourcentage en masse dans la composition de matière première du matériau d'aimant permanent à base de RTB ;
la teneur en Pr étant de 8,85-27,15 % en poids, telle que de 8,85 % en poids, 9,85 % en poids ; 10,15 % en poids, 10,85 % en poids, 11,85 % en poids, 12,15 % en poids, 13,15 % en poids, 14,15 % en poids, 16,15 % en poids, 17,15 % en poids, 18,15 % en poids, 19,15 % en poids, 20,15 % en poids, 21,15 % en poids, 22,15 % en poids, 23,15 % en poids, 24,15 % en poids, 25,15 % en poids ou 27,15 % en poids, le pourcentage faisant référence au pourcentage en masse dans la composition de matière première du matériau d'aimant permanent à base de RTB ;
R' comprenant en outre du Nd et/ou R, R étant un élément des terres rares outre Pr et Nd ; la teneur en Nd étant préférablement de 3,35-22,65 % en poids, plus préférablement de 3,35 % en poids, 5,35 % en poids, 6,65 % en poids, 6,85 % en poids, 7,35 % en poids, 7,85 % en poids, 8,35 % en poids, 8,65 % en poids, 8,85 % en poids, 9,35 % en poids, 10,65 % en poids, 10,85 % en poids, 11,35 % en poids, 11,65 % en poids, 11,85 % en poids, 12,35 % en poids, 12,65 % en poids ; 13,35 % en poids, 13,65 % en poids, 13,85 % en poids, 14,35 % en poids, 14,65 % en poids, 14,8 % en poids, 15,35 % en poids, 16,35 % en poids, 16,65 % en poids, 16,85 % en poids, 17,35 % en poids, 17,65 % en poids, 18,35 % en poids, 18,65 % en poids, 18,85 % en poids, 19,35 % en poids, 19,65 % en poids, 20,65 % en poids, 20,85 % en poids, 21,35 % en poids, 21,65 % en poids, 21,95 % en poids, 22,15 % en poids ou 22,65 % en poids, le pourcentage faisant référence au pourcentage en masse dans la composition de matière première du matériau d'aimant permanent à base de RTB ; le rapport en masse de Nd sur R' étant préférablement ≤ 0,72 ; la sorte de R étant préférablement Y et/ou Ce ; la teneur en R étant préférablement de 0 à 1 % en poids, par exemple 0,3 % en poids, le pourcentage faisant référence au pourcentage en masse dans la composition de matière première du matériau d'aimant permanent à base de RTB ;
R' comprenant en outre un élément lourd des terres rares RH ; la sorte de RH étant préférablement Dy et/ou Tb ; la teneur en RH étant préférablement 1,2-2,5 % en poids, telle que 1,2 % en poids, 1,5 % en poids, 2 % en poids ou 2,5 % en poids, et le pourcentage faisant référence au pourcentage en masse dans la composition de matière première du matériau d'aimant permanent à base de RTB ; le rapport en masse de RH sur R' étant préférablement < 0,253, par exemple 0,038-0,075, puis 0,038, 0,039, 0,046, 0,061 ou 0,075 ; lorsque le RH comprend du Tb, la teneur en Tb étant préférablement 1,2 à 2,0 % en poids, par exemple 1,2 % en poids, ou 2,0 % en poids, le pourcentage faisant référence au pourcentage en masse dans la composition de matière première du matériau d'aimant permanent à base de RTB ; lorsque le RH comprend du Dy, la teneur en Dy étant préférablement 1,5 à 2,5 % en poids, telle que 1,5 % en poids, 2,0 % en poids ou 2,5 % en poids, le pourcentage faisant référence au pourcentage en masse dans la composition de matière première du matériau d'aimant permanent à base de RTB ;
la teneur en B étant de 0,95-1,1 % en poids, telle que 0,95 % en poids, 0,96 % en poids, 0,98 % en poids ou 1,01 % en poids, le pourcentage faisant référence au pourcentage en masse dans la composition de matière première du matériau d'aimant permanent à base de RTB ;
la teneur en Fe étant de 61,5 à 69,5 % en poids, telle que de 61,79 % en poids, 61,89 % en poids, 62,44 % en poids, 62,89 % en poids, 63,24 % en poids, 63,84 % en poids, 63,87 % en poids, 63,94 % en poids, 64,99 % en poids, 66,19 % en poids, 66,29 % en poids, 66,47 % en poids, 66,52 % en poids, 66,55 % en poids, 66,61 % en poids, 66,69 % en poids, 66,75 % en poids, 66,85 % en poids, 66,97 % en poids, 67,00 % en poids, 67,02 % en poids, 67,068 % en poids, 67,13 % en poids, 67,14 % en poids, 67,19 % en poids, 67,24 % en poids ; 67,25 % en poids, 67,35 % en poids, 67,37 % en poids, 67,45 % en poids, 67,49 % en poids, 67,54 % en poids, 67,55 % en poids, 67,57 % en poids, 67,59 % en poids, 67,64 % en poids, 67,65 % en poids, 67,69 % en poids, 67,718 % en poids, 67,75 % en poids, 67,85 % en poids, 67,95 % en poids, 67,96 % en poids, 67,97 % en poids, 68,008 % en poids, 68,12 % en poids, 68,55 % en poids, 68,62 % en poids, 69,02 % en poids, 69,1 % en poids, 69,22 % en poids, 69,27 % en poids, 69,32 % en poids ou 69,45 % en poids, le pourcentage faisant référence au pourcentage en masse dans la composition de matière première du matériau d'aimant permanent à base de RTB ;
X étant Cu, Al, Ga, Co, Zr, Ti ou Nb, ou « Cu et Al », « Ga et Mn », « Cu, Al et Ga », « Cu, Al, Ga et Zr », « Cu, Al, Ga et Co » ou « Cu, Al, Ga, Zr et Co » ;
la teneur du X étant de 0 à 4,5 % en poids ; lorsque X comprend du Cu, la teneur du Cu étant préférablement de 0,2 à 0,5 % en poids ; lorsque le X comprend de l'AI, la teneur en Al étant préférablement de 0 à 0,8 % en poids, mais pas de 0, telle que 0,01-0,03 % en poids ou 0,5-0,8 % en poids ; lorsque le X comprend du Ga, la teneur en Ga étant préférablement de 0,0-1,85 % en poids, mais pas de 0, et plus préférablement de 0,1-1,55 % en poids ; lorsque le X comprend du Co, la teneur en Co étant préférablement de 0,0-3,0 % en poids, mais pas de 0, et plus préférablement de 0,5-2,5 % en poids ; lorsque le X comprend du Zr, la teneur en Zr étant préférablement de 0,25-0,35 % en poids ; lorsque le X comprend du Nb, la teneur en Nb étant préférablement de 0,25-0,35 % en poids ; lorsque le X comprend du Mn, la teneur en Mn étant préférablement de 0,0-0,03 % en poids, mais pas de 0 ; le pourcentage faisant référence au pourcentage en masse dans la composition de matière première du matériau d'aimant permanent à base de RTB ;
le matériau d'aimant permanent à base de RTB comprenant en outre M, M étant un ou plusieurs éléments parmi Ni, Zn, Ag, In, Sn, Bi, V, Cr, Hf, Ta et W ; la sorte de M étant préférablement Cr ; la teneur en M étant préférablement de 0 à 0,15 % en poids, mais pas de 0, et le pourcentage faisant référence au pourcentage en masse dans la composition de matière première du matériau d'aimant permanent à base de RTB.

3. Procédé de préparation d'un matériau d'aimant permanent à base de RTB selon la revendication 1 ou 2, pendant le processus de pulvérisation, la teneur en oxygène O dans l'atmosphère de pulvérisation étant de 0 à 50 ppm, telle que de 0 ppm, 5 ppm, 10 ppm, 15 ppm, 20 ppm, 25 ppm, 30 ppm, 35 ppm, 40 ppm, 45 ppm, ou 50 ppm ;
le dispersant étant un lubrifiant et/ou un antioxydant, préférablement le lubrifiant étant le stéarate de zinc ; lorsque le dispersant contient du stéarate de zinc, la quantité de stéarate de zinc pouvant être de 0,04-0,14 %, telle que de 0,04 %, 0,05 %, 0,06 %, 0,07 %, 0,08 %, 0,09 %, 0,1 %, 0,11 %, 0,12 %, 0,13 % ou 0,14 %, le pourcentage faisant référence au pourcentage en masse par rapport à la masse totale de la poudre mélangée ;
la teneur du dispersant étant de 0,04-0,14 %, telle que de 0,04 %, 0,05 %, 0,06 %, 0,07 %, 0,08 %, 0,09 %, 0,1 %, 0,11 %, 0,12 %, 0,13 % ou 0,14 %, le pourcentage faisant référence au pourcentage en masse par rapport à la masse totale de la poudre mélangée ;
pendant le processus de pressage, la teneur en oxygène O dans l'atmosphère de pressage étant de 10 à 30 ppm, telle que de 10 ppm, 12 ppm, 14 ppm, 16 ppm, 18 ppm, 20 ppm, 22 ppm, 24 ppm, 26 ppm, 28 ppm ou 30 ppm.
